



US008962907B2

(12) **United States Patent**  
**Hanada et al.**

(10) **Patent No.:** **US 8,962,907 B2**  
(45) **Date of Patent:** **Feb. 24, 2015**

(54) **METHOD FOR REMOVING RADIOACTIVE CESIUM, HYDROPHILIC RESIN COMPOSITION FOR REMOVING RADIOACTIVE CESIUM, METHOD FOR REMOVING RADIOACTIVE IODINE AND RADIOACTIVE CESIUM, AND HYDROPHILIC RESIN COMPOSITION FOR REMOVING RADIOACTIVE IODINE AND RADIOACTIVE CESIUM**

(71) Applicants: **Dainichiseika Color & Chemicals Mfg. Co., Ltd.**, Tokyo (JP); **Ukima Chemicals & Color Mfg. Co., Ltd.**, Tokyo (JP)

(72) Inventors: **Kazuyuki Hanada**, Tokyo (JP); **Manabu Uruno**, Tokyo (JP); **Kazuya Kimura**, Tokyo (JP); **Kenichi Takahashi**, Tokyo (JP)

(73) Assignees: **Dainichiseika Color & Chemicals Mfg. Co., Ltd.**, Chuo-Ku (JP); **Ukima Chemicals & Color Mfg. Co., Ltd.**, Chuo-Ku (JP)

(\*) Notice: Subject to any disclaimer, the term of this patent is extended or adjusted under 35 U.S.C. 154(b) by 0 days.

(21) Appl. No.: **14/300,291**

(22) Filed: **Jun. 10, 2014**

(65) **Prior Publication Data**

US 2014/0288346 A1 Sep. 25, 2014

**Related U.S. Application Data**

(63) Continuation of application No. PCT/JP2013/050980, filed on Jan. 18, 2013.

(30) **Foreign Application Priority Data**

Jan. 18, 2012 (JP) ..... 2012-007662  
Feb. 7, 2012 (JP) ..... 2012-023592  
Mar. 23, 2012 (JP) ..... 2012-067619  
Apr. 9, 2012 (JP) ..... 2012-088298

(51) **Int. Cl.**

**G21F 9/12** (2006.01)  
**G21F 9/16** (2006.01)  
**G21F 9/30** (2006.01)

(52) **U.S. Cl.**  
CPC **G21F 9/167** (2013.01); **G21F 9/12** (2013.01);  
**G21F 9/307** (2013.01); **Y10S 588/901**  
(2013.01)

USPC ..... **588/8**; 588/412; 588/901  
(2013.01)  
(58) **Field of Classification Search**  
USPC ..... 588/6, 8, 315, 410, 412, 901  
See application file for complete search history.

(56) **References Cited**

**U.S. PATENT DOCUMENTS**

2004/0178385 A1 9/2004 Bispo et al.

**FOREIGN PATENT DOCUMENTS**

|    |                |        |
|----|----------------|--------|
| EP | 0 475 635 A1   | 3/1992 |
| JP | 62-044239 B2   | 9/1987 |
| JP | 02-047599 A1   | 2/1990 |
| JP | 04-118596 A1   | 4/1992 |
| JP | 04-243543 A1   | 8/1992 |
| JP | 06-138298 A1   | 5/1994 |
| JP | 2005-500158 A1 | 1/2005 |
| JP | 2005-037133 A1 | 2/2005 |
| JP | 2008-116280 A1 | 5/2008 |

**OTHER PUBLICATIONS**

International Search Report (Application No. PCT/JP2013/050980) dated Feb. 12, 2013.

Japanese Office Action (Application No. 2012-023592) dated Nov. 4, 2014.

*Primary Examiner* — Edward Johnson

(74) *Attorney, Agent, or Firm* — Burr & Brown, PLLC

(57) **ABSTRACT**

The present invention intends to provide a method for removing radioactive cesium, or radioactive iodine and radioactive cesium that is simple and low-cost, further does not require an energy source such as electricity, moreover can take in and stably immobilize the removed radioactive substances within a solid, and can reduce the volume of radioactive waste as necessary, and to provide a hydrophilic resin composition using for the method for removing radioactive cesium, or radioactive iodine and radioactive cesium, and the object of the present invention is achieved by using a hydrophilic resin composition containing: at least one hydrophilic resin selected from the group consisting of a hydrophilic polyurethane resin, a hydrophilic polyurea resin, and a hydrophilic polyurethane-polyurea resin each having at least a hydrophilic segment; and a zeolite dispersed therein in a ratio of at least 1 to 200 mass parts relative to 100 mass parts of the hydrophilic resin.

**23 Claims, 5 Drawing Sheets**

Figure 1



Figure 2



Figure 3



Figure 4



Figure 5



Figure 6



Figure 7



Figure 8



Figure 9



**METHOD FOR REMOVING RADIOACTIVE CESIUM, HYDROPHILIC RESIN COMPOSITION FOR REMOVING RADIOACTIVE CESIUM, METHOD FOR REMOVING RADIOACTIVE IODINE AND RADIOACTIVE CESIUM, AND HYDROPHILIC RESIN COMPOSITION FOR REMOVING RADIOACTIVE IODINE AND RADIOACTIVE CESIUM**

**TECHNICAL FIELD**

The present invention relates to a removal method capable of applying removal processing to radioactive cesium in a radioactive waste liquid and/or a radioactive solid matter generated from a nuclear power plant or a reprocessing facility of spent nuclear fuel, and to a hydrophilic resin composition suitable for the method, the hydrophilic resin composition exhibiting a function of immobilizing radioactive cesium. The present invention also relates to a removal method capable of applying removal processing to both of radioactive iodine and radioactive cesium present in a radioactive waste liquid and/or a radioactive solid matter generated from a nuclear power plant or a reprocessing facility of spent nuclear fuel, and to a hydrophilic resin composition exhibiting a function of immobilizing both of the radioactive iodine and the radioactive cesium.

**BACKGROUND ART**

In currently widespread nuclear reactor power plants, nuclear fission in a nuclear reactor is accompanied by generation of a considerable amount of radioactive by-products. The main radioactive substances among the radioactive by-products are fission products and active elements including extremely dangerous radioactive isotopes such as radioactive iodine, radioactive cesium, radioactive strontium, and radioactive cerium. Since radioactive iodine among these radioactive substances turns into a gas at 184°C., there is a risk that the radioactive iodine is extremely liable to be discharged at the time of inspection or exchange of nuclear fuel and furthermore by an unforeseen event such as an accident during handling nuclear fuel or a reactor excursion accident. The major radioactive iodine isotopes to be taken into account at the time of discharge are iodine 129 having a long half-life (half-life:  $1.57 \times 10^7$  years) and iodine 131 having a short half-life (half-life: 8.05 days). Here, ordinary iodine that does not exhibit radioactivity is an essential trace element in the human body, is collected in the thyroid gland near the throat, and becomes a component of a growth hormone. Therefore, when a human takes in radioactive iodine through breathing or water/foods, the radioactive iodine is collected in the thyroid gland in the same way as in the case of ordinary iodine and increases internal exposure to radioactivity, and accordingly, a particularly strict measure for reducing the amount of radioactivity to be discharged must be implemented with regard to radioactive iodine.

Moreover, radioactive cesium has a melting point of 28.4°C., is one of metals that become liquid at around a normal temperature, and is a metal that is extremely liable to be discharged as well as radioactive iodine. The major radioactive cesium isotopes to be taken into account at the time of discharge are cesium 134 having a relatively short half-life (half-life: 2 years) and cesium 137 having a long half-life (half-life: 30 years). Among the major radioactive cesium isotopes, cesium 137 in particular not only has a long half-life but also emits high-energy radiation, and has a property that

water solubility is high because the radioactive cesium is an alkaline metal. Furthermore, radioactive cesium is easily absorbed in the human body through breathing and also through skin and is uniformly dispersed in the whole body, and therefore a health hazard to humans when the radioactive cesium is discharged becomes serious.

Thus, when radioactive cesium is accidentally discharged due to an unforeseen event or the like from nuclear reactors in operation all over the world, there are concerns that the radioactive cesium causes not only radioactive contamination to workers at nuclear reactors or neighborhood residents but also radioactive contamination over a wider range to humans and animals through foods or water contaminated by the radioactive cesium carried by air. The danger with regard to the radioactive contamination has already been proven undoubtedly by the accident in Chernobyl nuclear power plant.

To such a situation, a cleaning processing system, a physical/chemical processing system by solid adsorbent filling using fibrous activated carbon or the like (see Patent Literatures 1 and 2), processing by an ion exchange material (see Patent Literature 3), and so on have been studied as a method for processing radioactive iodine generated in a nuclear reactor.

However, any of the above methods has problems as described below, and the development of a method for removing radioactive iodine in which these problems are solved is desired. First of all, an alkaline cleaning method or the like exists as a cleaning processing system practically used, however there are lots of problems in terms of quantity and safety to apply processing by the cleaning processing system with a liquid adsorbent and store the processed liquid as it is for a long period of time. Moreover, in the physical/chemical processing system by solid adsorbent filling, captured radioactive iodine is always facing the possibility of being replaced with other gases, and moreover the processing system has a problem that an adsorbed matter is liable to be discharged when the temperature increases. Furthermore, in the processing system by an ion exchange material, the heat resistant temperature of the ion exchange material is up to about 100°C. and there is a problem that the ion exchange material cannot exhibit sufficient performance at a temperature higher than the heat resistant temperature.

On the other hand, as a method for removing processing of radioactive cesium generated by nuclear fission in a nuclear reactor, an adsorption method with an inorganic ion exchanger or a selective ion exchange resin, a coprecipitation method by using a heavy metal and a soluble ferrocyanide or ferrocyanide salt together, a chemical processing method with a cesium precipitation reagent, and so on are known (see, for example, Patent Literature 4).

However, in any of the above-described processing methods, large scale facilities such as a circulation pump, a cleaning tank, and furthermore a filling tank containing various adsorbents are necessary, and in addition, a large amount of energy to operate these facilities is needed. Moreover, when supply of the power source is suspended as in the accident occurred at the Fukushima No. 1 nuclear power plant in Japan on Mar. 11, 2011, these facilities cannot be operated and, in such a case, the degree of contamination risk by radioactive cesium increases. And particularly in the case where the supply of the power source is suspended, applying a method for removing radioactive cesium diffused into peripheral areas by a reactor excursion accident falls into an extremely difficult situation, and it is concerned that a situation in which radioactive contamination expands may occur. Accordingly, there is an urgent need to develop a method for removing

radioactive cesium that is applicable even when the situation in which the supply of the power source is suspended occurs, and when such method for removing radioactive cesium is developed, the method is extremely useful.

## CITATION LIST

## Patent Literature

- Patent Literature 1: JP-62-44239  
 Patent Literature 2: JP-A-2008-116280  
 Patent Literature 3: JP-A-2005-37133  
 Patent Literature 4: JP-A-4-118596

## SUMMARY OF INVENTION

## Technical Problem

Accordingly, an object of the first present invention and the second present invention is to solve the problems of conventional arts and to provide a novel method for removing radioactive cesium that is simple and low-cost, furthermore does not require an energy source such as electricity, moreover can take in and stably immobilize the removed radioactive cesium within a solid, and is capable of reducing the volume of radioactive waste as necessary. Moreover, another object of the first present invention and the second present invention is to provide a novel hydrophilic resin composition that has a function useful for the above-described method and is capable of immobilizing radioactive cesium, the hydrophilic resin composition capable of realizing applying removal processing to radioactive cesium simply.

Furthermore, yet another object of the second present invention is to provide a novel hydrophilic resin composition for removing radioactive cesium excellent in practical use by which hydrophilic resin composition the water resistance and the blocking resistance performance (sticking resistance) of the surface are improved in the case where the hydrophilic resin composition is used in a form such as a resin film or sheet in applying processing in addition to having a function particularly useful for the above-described method and capable of immobilizing radioactive cesium.

Moreover, an object of the third present invention and the fourth present invention is, in providing an effective removal method capable of applying processing to radioactive iodine and radioactive cesium together, to solve the problems of conventional arts and to provide a novel method for removing radioactive iodine and radioactive cesium that is simple and low-cost, furthermore does not require an energy source such as electricity, moreover can take in and stably immobilize the removed radioactive iodine and the radioactive cesium within a solid, and is capable of reducing the volume of radioactive waste as necessary. Moreover, another object of the third present invention and the fourth present invention is to provide a novel hydrophilic resin composition that has a function useful in carrying out the above-described method and is capable of immobilizing both of radioactive iodine and radioactive cesium, the hydrophilic resin composition capable of applying removal processing to these radioactive substances together.

Furthermore, yet another object of the fourth present invention is to provide a novel hydrophilic resin composition more excellent in practical use by which hydrophilic resin composition the water resistance and the blocking resistance performance (sticking resistance) of the surface are improved in the case where the hydrophilic resin composition is used in a form such as a resin film or sheet in applying processing in

addition to having a function particularly useful for the above-described method and capable of immobilizing radioactive iodine and radioactive cesium.

## Solution to Problem

Each of the objects is achieved by the first, the second, the third, or the fourth present invention described below. Namely, as the first present invention, provided is a method 10 for removing radioactive cesium applying removal processing to radioactive cesium in a radioactive waste liquid and/or a radioactive solid matter using a hydrophilic resin composition comprising a hydrophilic resin and a zeolite, wherein the hydrophilic resin composition comprises at least one hydrophilic resin selected from the group consisting of a hydrophilic polyurethane resin, a hydrophilic polyurea resin, and a hydrophilic polyurethane-polyurea resin each having a hydrophilic segment; and the hydrophilic resin composition comprises the zeolite dispersed therein in a ratio of at least 1 15 to 200 mass parts relative to 100 mass parts of the hydrophilic resin.

As the second present invention, provided is a method for removing radioactive cesium applying removal processing to radioactive cesium present in a radioactive waste liquid and/or a radioactive solid matter using a hydrophilic resin composition comprising a hydrophilic resin and a zeolite, wherein the hydrophilic resin comprises at least one selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a polysiloxane segment; and the hydrophilic resin composition comprises the zeolite dispersed therein in a ratio of at least 1 to 200 mass parts relative to 100 mass parts of the hydrophilic resin.

In the above-described second present invention, it is preferable that the hydrophilic resin in the hydrophilic resin composition is a resin formed from, as a part of a raw material, a compound having at least one active hydrogen-containing group and a polysiloxane segment in the same molecule.

As another embodiment of the first present invention, provided is a hydrophilic resin composition for removing radioactive cesium having a function capable of immobilizing radioactive cesium in liquid and/or a solid matter, wherein the hydrophilic resin composition comprises a hydrophilic resin and a zeolite; the hydrophilic resin is a resin having a hydrophilic segment, the resin being insoluble to water and hot water; and the zeolite is dispersed in the hydrophilic resin composition in a ratio of at least 1 to 200 mass parts relative to 100 mass parts of the hydrophilic resin.

As yet another embodiment of the first present invention, provided is a hydrophilic resin composition for removing radioactive cesium having a function capable of immobilizing radioactive cesium in liquid and/or a solid matter, wherein the hydrophilic resin composition comprises a hydrophilic resin and a zeolite; the hydrophilic resin is at least one selected from the group consisting of a hydrophilic polyurethane resin, a hydrophilic polyurea resin, and a hydrophilic polyurethane-polyurea resin each having a hydrophilic segment and each obtained by reacting an organic polyisocyanate with a high molecular weight hydrophilic polyol and/or polyamine being a hydrophilic component; and the zeolite is dispersed in the hydrophilic resin composition in a ratio of at least 1 to 200 mass parts relative to 100 mass parts of the hydrophilic resin.

As another embodiment of the second present invention, provided is a hydrophilic resin composition for removing

radioactive cesium exhibiting a function capable of immobilizing radioactive cesium in liquid and/or a solid matter, wherein the hydrophilic resin composition comprises a hydrophilic resin and a zeolite; the hydrophilic resin is a resin having a hydrophilic segment and a polysiloxane segment and obtained by reacting, as a part of a raw material, a compound having at least one active hydrogen-containing group and a polysiloxane segment in the same molecule, the resin being insoluble to water and hot water; and the zeolite is dispersed in the hydrophilic resin composition in a ratio of at least 1 to 200 mass parts relative to 100 mass parts of the hydrophilic resin.

As yet another embodiment of the second present invention, provided is a hydrophilic resin composition for removing radioactive cesium exhibiting a function capable of immobilizing radioactive cesium in liquid and/or a solid matter, wherein the hydrophilic resin composition comprises a hydrophilic resin and a zeolite; the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a polysiloxane segment, and each obtained by reacting an organic polyisocyanate, a high molecular weight hydrophilic polyol and/or polyamine being a hydrophilic component, and a compound having at least one active hydrogen-containing group and a polysiloxane segment in the same molecule; and the zeolite is dispersed in the hydrophilic resin composition in a ratio of at least 1 to 200 mass parts relative to 100 mass parts of the hydrophilic resin.

Preferable embodiments of the first or the second present invention relating to the above-described method for removing radioactive cesium or the hydrophilic resin composition include: the hydrophilic segment is a polyethylene oxide segment; and the zeolite is a compound represented by the following general formula (1).



[Where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number of from 1 to 18, and  $n$  is a number of from 1 to 70]

As the third present invention, provided is a method for removing radioactive iodine and radioactive cesium applying removal processing to both of radioactive iodine and radioactive cesium in a radioactive waste liquid and/or a radioactive solid matter using a hydrophilic resin composition comprising a hydrophilic resin and a zeolite, wherein the hydrophilic resin comprises at least one hydrophilic resin selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a tertiary amino group; and the hydrophilic resin composition comprises the zeolite dispersed therein in a ratio of at least 1 to 200 mass parts relative to 100 mass parts of the hydrophilic resin.

A preferable embodiment of the above-described third present invention includes that the hydrophilic resin is a resin formed from, as a part of a raw material, a polyol having at least one tertiary amino group or a polyamine having at least one tertiary amino group.

As the fourth present invention, provided is a method for removing radioactive iodine and radioactive cesium applying removal processing to both of radioactive iodine and radioactive cesium present in a radioactive waste liquid and/or a radioactive solid matter using a hydrophilic resin composition comprising a hydrophilic resin and a zeolite, wherein the

hydrophilic resin comprises at least one selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a tertiary amino group and a polysiloxane segment; and the zeolite is dispersed in the hydrophilic resin composition in a ratio of at least 1 to 200 mass parts relative to 100 mass parts of the hydrophilic resin.

A preferable embodiment of the above-described fourth present invention includes that the hydrophilic resin is a resin formed from, as a part of a raw material, a polyol having at least one tertiary amino group or a polyamine having at least one tertiary amino group, and a compound having at least one active hydrogen-containing group and a polysiloxane segment in the same molecule.

As another embodiment of the third present invention, provided is a hydrophilic resin composition for removing radioactive iodine and radioactive cesium exhibiting a function capable of immobilizing both of radioactive iodine and radioactive cesium in liquid and/or a solid matter, wherein the hydrophilic resin composition comprises a hydrophilic resin and a zeolite; the hydrophilic resin is a resin having a hydrophilic segment, having, in the molecular chain, a tertiary amino group, and formed from, as a part of a raw material, a polyol having at least one tertiary amino group or a polyamine having at least one tertiary amino group, the resin being insoluble to water and hot water; and the zeolite is dispersed in the hydrophilic resin composition in a ratio of at least 1 to 200 mass parts relative to 100 mass parts of the hydrophilic resin.

As yet another embodiment of the third present invention, provided is a hydrophilic resin composition for removing radioactive iodine and radioactive cesium having a function capable of immobilizing both of radioactive iodine and radioactive cesium in liquid and/or a solid matter, wherein the hydrophilic resin composition comprises a hydrophilic resin and a zeolite; the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a tertiary amino group, and each obtained by reacting an organic polyisocyanate, a high molecular weight hydrophilic polyol and/or polyamine being a hydrophilic component, and a compound having at least one active hydrogen-containing group and at least one tertiary amino group in the same molecule; and the zeolite is dispersed in the hydrophilic resin composition in a ratio of at least 1 to 200 mass parts relative to 100 mass parts of the hydrophilic resin.

As another embodiment of the fourth present invention, provided is a hydrophilic resin composition for removing radioactive iodine and radioactive cesium exhibiting a function capable of immobilizing both of radioactive iodine and radioactive cesium in liquid and/or a solid matter, wherein the hydrophilic resin composition comprises a hydrophilic resin and a zeolite; the hydrophilic resin is a resin having a hydrophilic segment, having, in the molecular chain, a tertiary amino group and a polysiloxane segment, and obtained by reacting a polyol having at least one tertiary amino group or a polyamine having at least one tertiary amino group with a compound having at least one active hydrogen-containing group and a polysiloxane segment in the same molecule, the resin being insoluble to water and hot water; and the zeolite is

dispersed in the hydrophilic resin composition in a ratio of at least 1 to 200 mass parts relative to 100 mass parts of the hydrophilic resin.

As yet another embodiment of the fourth present invention, provided is a hydrophilic resin composition for removing radioactive iodine and radioactive cesium exhibiting a function capable of immobilizing both of radioactive iodine and radioactive cesium in liquid and/or a solid matter, wherein the hydrophilic resin composition comprises a hydrophilic resin and a zeolite; the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a tertiary amino group and a polysiloxane segment, and each obtained by reacting an organic polyisocyanate, a high molecular weight hydrophilic polyol and/or polyamine being a hydrophilic component, a compound having at least one active hydrogen-containing group and at least one tertiary amino group in the same molecule, and a compound having at least one active hydrogen-containing group and a polysiloxane segment in the same molecule; and the zeolite is dispersed in the hydrophilic resin composition in a ratio of at least 1 to 200 mass parts relative to 100 mass parts of the hydrophilic resin.

Preferable embodiments of the third or the fourth present invention relating to the above-described method for removing radioactive cesium or the hydrophilic resin composition include: the hydrophilic segment is a polyethylene oxide segment; and the zeolite is a compound represented by the following general formula (1).



[Where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number of from 1 to 18, and  $n$  is a number of from 1 to 70]

#### Advantageous Effects of Invention

According to the first present invention or the second present invention, provided is a novel method for removing radioactive cesium that is capable of applying processing to radioactive cesium present in liquid or a solid matter simply and at low cost, furthermore does not require an energy source such as electricity, moreover can take in and stably immobilize the removed radioactive cesium within a solid, and can achieve the volume reduction of radioactive waste as necessary.

According to the first present invention, provided is a novel hydrophilic resin composition that has a function capable of immobilizing radioactive cesium, makes it possible to realize applying removal processing to radioactive cesium, and can reduce the volume of radioactive waste as necessary because the main component of the hydrophilic resin composition is a resin composition. The remarkable effects of the present invention are achieved by an extremely simple method that utilizes the hydrophilic resin composition comprising a zeolite dispersed in a hydrophilic resin having a hydrophilic segment in the structure thereof. The above-described hydrophilic resin is obtained by reacting, for example, an organic polyisocyanate with a high molecular weight hydrophilic polyol and/or polyamine (hereinafter, each of the polyol and the polyamine is referred to as a "hydrophilic component"), and, more specifically, examples of the hydrophilic resin include at least one selected from the group consisting of a hydrophilic polyurethane resin, a hydrophilic polyurea resin, and a hydrophilic polyurethane-polyurea resin.

Particularly, according to the second present invention, provided is a hydrophilic resin composition with high practicability that has a function capable of immobilizing radioactive cesium and realizes improvement in the water resistance and the blocking resistance (sticking resistance) of the surface when used in a form such as a film form at the time of removing processing, and thereby the removing processing of radioactive cesium can be realized in a better state. Furthermore, since the main component of the hydrophilic resin 10 composition is a resin composition, a novel hydrophilic resin composition capable of also reducing the volume of radioactive waste as necessary is provided. These remarkable effects in the second present invention are achieved by an extremely simple method that utilizes a hydrophilic resin composition 15 comprising a zeolite dispersed therein together with a hydrophilic resin having a hydrophilic segment in the structure thereof and having, in the main chain and/or a side chain, a polysiloxane segment. The hydrophilic resin that characterizes the second present invention is obtained by reacting, for 20 example, an organic polyisocyanate, a hydrophilic component, and a compound having at least one active hydrogen-containing group and a polysiloxane segment in the same molecule, and more specific examples of the hydrophilic resin include at least one selected from the group consisting of 25 a hydrophilic polyurethane resin, a hydrophilic polyurea resin, and a hydrophilic polyurethane-polyurea resin each having the above-described structure.

According to the third present invention or the fourth present invention, provided is a novel method that is capable 30 of applying processing to radioactive iodine and radioactive cesium present in liquid or a solid matter simply and at low cost, furthermore does not require an energy source such as electricity, moreover can take in, fix and further stably immobilize the removed radioactive iodine and the removed radioactive cesium within a solid, can achieve the volume reduction 35 of radioactive waste as necessary, and can apply removing processing of radioactive iodine and radioactive cesium together. According to the present invention, provide is a novel hydrophilic resin composition that has a function 40 capable of immobilizing both of radioactive iodine and radioactive cesium, makes it possible to realize applying removal processing to radioactive iodine and radioactive cesium together, and can reduce the volume of radioactive waste as necessary because the main component of the hydrophilic 45 resin composition is a resin composition.

The remarkable effects in the third present invention are achieved by an extremely simple method that utilizes a hydrophilic resin composition obtained by dispersing a zeolite in a hydrophilic resin such as a hydrophilic polyurethane resin, a hydrophilic polyurea resin, and a hydrophilic polyurethane-polyurea resin obtained by reacting an organic polyisocyanate, a hydrophilic component, and a compound having at least 50 one active hydrogen-containing group and at least one tertiary amino group in the same molecule.

Particularly, according to the fourth present invention, provided is a hydrophilic resin composition with high practicability that has a function of immobilizing radioactive iodine and radioactive cesium and realizes improvement in the water resistance and the blocking resistance performance (sticking 55 resistance) of the surface when used in a form such as a film form at the time of removing processing, and thereby the removing processing of radioactive iodine and radioactive cesium can be realized in a better state. The remarkable effects in the fourth present invention are achieved by the 60 hydrophilic resin having a hydrophilic segment in the structure thereof, and having, in the molecular chain, at least one tertiary amino group and a polysiloxane segment, and in more 65

detail, the remarkable effects in the fourth present invention are achieved by an extremely simple method that utilizes a hydrophilic resin composition obtained by dispersing a zeolite in a hydrophilic resin such as a hydrophilic polyurethane resin, a hydrophilic polyurea resin, and a hydrophilic polyurethane-polyurea resin obtained by reacting an organic polyisocyanate, a hydrophilic component, a compound having at least one active hydrogen-containing group and at least one tertiary amino group in the same molecule, and a compound having at least one active hydrogen-containing group and a polysiloxane segment in the same molecule.

#### BRIEF DESCRIPTION OF DRAWINGS

FIG. 1 is a graph showing the relation between the cesium concentration in each aqueous solution and the immersion time of each film comprising a hydrophilic resin composition of Examples 1-1 to 1-3 relating to the first present invention.

FIG. 2 is a graph showing the relation between the cesium concentration of each aqueous solution and the immersion time of each film comprising a hydrophilic resin composition of Examples 2-1 to 2-3 relating to the second present invention.

FIG. 3 is a graph showing the relation between the cesium concentration in each aqueous solution and the immersion time of each film comprising a non-hydrophilic resin composition of Comparative Examples 1A and 2A to the first present invention and Comparative Examples 1a and 2a to the second present invention.

FIG. 4 is a graph showing the relation between the iodine concentration of each aqueous solution and the immersion time of each film prepared by a hydrophilic resin composition of Examples 3-1 to 3-3 relating to the third present invention.

FIG. 5 is a graph showing the relation between the cesium concentration of each aqueous solution and the immersion time of each film prepared by a hydrophilic resin composition of Examples 3-1 to 3-3 relating to the third present invention.

FIG. 6 is a graph showing the relation between the iodine concentration of each aqueous solution and the immersion time of each film prepared by a hydrophilic resin composition of Examples 4-1 to 4-3 relating to the fourth present invention.

FIG. 7 is a graph showing the relation between the cesium concentration of each aqueous solution and the immersion time of each film prepared by a hydrophilic resin composition of Examples 4-1 to 4-3 relating to the fourth present invention.

FIG. 8 is a graph showing the relation between the iodine concentration of each aqueous solution and the immersion time of each film prepared by a non-hydrophilic resin composition of Comparative Examples 1b to 2b to the third present invention and the fourth present invention.

FIG. 9 is a graph showing the relation between the cesium concentration of each aqueous solution and the immersion time of each film prepared by a non-hydrophilic resin composition of Comparative Examples 1b to 2b to the third present invention and the fourth present invention.

#### DESCRIPTION OF EMBODIMENTS

Next, each of the first present invention to the fourth present invention will be described in more detail giving preferable embodiments.

The first present invention and the second present invention relate to a method for removing radioactive cesium, and the main characteristic is to use a hydrophilic resin composition capable of immobilizing radioactive cesium, the hydrophilic

resin composition comprising a zeolite dispersed in a hydrophilic resin having a particular structure.

Moreover, the third present invention and the fourth present invention relate to a method for removing radioactive iodine and radioactive cesium, and the main characteristic is to use a hydrophilic resin composition capable of immobilizing both of radioactive iodine and radioactive cesium, the hydrophilic resin composition comprising a zeolite dispersed in a hydrophilic resin having a particular structure.

Here, the "hydrophilic resin" in the present invention means a resin that has a hydrophilic group in the molecule thereof but is insoluble to water, hot water, and so on, and the hydrophilic resin in the present invention is clearly distinguished from a water soluble resin such as polyvinyl alcohols, polyvinyl pyrrolidones, polyacrylic acids, and cellulose derivatives.

Each of the hydrophilic resin compositions that characterize the first present invention to the fourth present invention comprises a hydrophilic resin having a particular structure and a zeolite, and radioactive cesium can favorably be removed from radioactive waste liquid or a radioactive solid matter in the case where any of the hydrophilic resin compositions is used. The present inventors consider as follows with regard to the reason why it becomes possible to remove radioactive cesium by using these hydrophilic resin compositions. First of all, any of the hydrophilic resins used in the first present invention to the fourth present invention has a hydrophilic segment in the structure thereof and therefore exhibits excellent water absorbency due to the presence of the hydrophilic segment. For this reason, it is considered that ionized radioactive cesium that is an object of processing is quickly taken in the resin. And in any of the removal methods of the first present invention to the fourth present invention, the hydrophilic resin composition comprising a zeolite dispersed in a hydrophilic resin that exhibits such a water-absorbing function is used, and, as described later, it is known that selective adsorption or the like of a cesium ion occurs on the zeolite and the zeolite can be utilized for the removal of the cesium ion. It is considered that since the above-described hydrophilic resin capable of quickly taking in ionized radioactive cesium that is an object of processing and the zeolite are present together in any of the hydrophilic resin compositions that characterize the present invention, radioactive cesium is fixed to the dispersed zeolite more quickly and more effectively and immobilized by the resin, and, as a result thereof, the effective removal of radioactive cesium can be achieved in the first present invention to the fourth present invention. In addition, according to the third present invention and the fourth present invention in which the resins the structures of which are different from the structures of the resins used in the first present invention and the second present invention are used as a hydrophilic resin, it becomes possible to apply removing processing to not only radioactive cesium as described above, but also both of radioactive iodine and radioactive cesium, however the reason for this will be described later.

#### [Zeolite]

A zeolite used in the present invention can be synthesized artificially but is a crystalline compound: comprising silicon, aluminum, and oxygen; having fine pores of a molecular level; and being produced naturally, and zeolites having various crystalline structures are known. Since the zeolite has a particular crystalline structure with pores having a very large surface area, the zeolite exhibits high adsorbing ability to gases, ions, or the like and high catalytic activity promoting various chemical reactions, and further, since sieving of mol-

## 11

ecules by the size of the pores can be performed, the zeolite has been used in a broad range of industrial fields.

A natural zeolite is a mineral having voids (pores) as described above in the crystalline structure among alumino-silicates represented by the general formula (1).



[Where, in the formula (1),  $M^{2+}$  is any one of  $Ca^{2+}$ ,  $Mn^{2+}$ ,  $Ba^{2+}$ , and  $Mg^{2+}$ ,  $M^{+}$  is any one of  $Na^{+}$ ,  $K^{+}$ , and  $Li^{+}$ ,  $m$  is a number of from 1 to 18, and  $n$  is a number of from 1 to 70].

The zeolite is widely used as a catalyst and an adsorbing material as described above and, in addition, since a cation contained in the zeolite can easily be exchanged to another ion and therefore the zeolite exhibits a high ion exchange property, and further, since the zeolite can be used even under the condition of a high temperature that is not suitable for a resin, the zeolite is also useful as an ion exchange material. In the present invention, by utilizing the high ion exchange property in particular that the zeolite has in addition to the afore-mentioned high adsorbing function that the zeolite has, radioactive cesium present in liquid and/or a solid matter is removed. Here, the ion exchange property that the zeolite has is specifically described. The ion exchange property that the zeolite has is exhibited due to the crystalline structure that forms a skeleton of the zeolite as described below. Since silicon (Si) as one component that makes a skeleton of the zeolite (crystal lattice) is a four-valent cation, the balance of electrical charges are kept between silicon and oxygen that is a divalent anion in the composition of  $SiO_2$ , however since aluminum (Al) that is another component is a trivalent cation, when aluminum is incorporated in the skeleton in place of silicon, one positive charge runs short and a deficit of a cation occurs. Therefore, another cation is contained in the zeolite and the balance of charges is kept by incorporating a cation such as sodium (Na), calcium (Ca), potassium (K), or the like in the part where the deficiency occurs. Since the cation incorporated and contained in the zeolite has a property that the cation is replaced with another cation and vice versa, the zeolite has a high ion exchange property. Here, the order of priority of the cation exchange that the zeolite has is as follows.

## &lt;Ion Exchange Order&gt;

Cesium (Cs)>rubidium (Rb)>ammonium ( $NH_4$ )>barium (Ba)>strontium (Sr)>sodium (Na)>calcium (Ca)>iron (Fe)>aluminum (Al)>magnesium (Mg)>lithium (Li)

As described above, since the ion exchange order of cesium and strontium is high, it is considered that the ion exchange property that the zeolite has can be utilized for removing radioactive substances such as radioactive cesium, and this is publicly known. In the first present invention to the fourth present invention, methods capable of applying removal processing to radioactive cesium more efficiently, simply, and economically are provided by using a hydrophilic resin composition comprising the zeolite dispersed in a hydrophilic resin. Above all, in the second present invention and the fourth present invention, methods more excellent in practicability by which methods radioactive cesium can be quickly taken in and removing processing can be applied to radioactive cesium further more efficiently, simply, and economically are provided by using a hydrophilic resin composition obtained by dispersing a zeolite in a hydrophilic resin having a particular structure, the hydrophilic resin allowing the water resistance and the blocking resistance of the surface to

## 12

improve in the case where the hydrophilic resin composition is used as a film or the like. Hereinafter, each hydrophilic resin that constitutes the first present invention to the fourth present invention will be described in detail.

5 [Hydrophilic Resin]  
(First Hydrophilic Resin)

The hydrophilic resin that characterizes the first present invention (hereinafter, referred to as the first hydrophilic resin) has a characteristic of having a hydrophilic segment comprising a hydrophilic component as a constituent unit. Namely, the first hydrophilic resin may comprise at least one hydrophilic resin selected from the group consisting of hydrophilic resins such as a hydrophilic polyurethane resin, a hydrophilic polyurea resin, and a hydrophilic polyurethane-polyurea resin each having a hydrophilic segment comprising a hydrophilic component as a constituent unit in the structure thereof. Each hydrophilic segment in these hydrophilic resins is randomly bonded through a urethane bond, a urea bond, a urethane-urea bond, or the like in the case where a chain extender is not used at the time of synthesizing the hydrophilic resin. Moreover, in the case where the chain extender is used at the time of synthesizing the hydrophilic resin, the structure is made so that a short chain that is a residue of the chain extender is present, together with the above-described bonds, between the above-described bonds.

Furthermore, the first hydrophilic resin composition that can be utilized for the method for removing radioactive cesium in the first present invention (hereinafter, referred to as the first hydrophilic resin composition) has a characteristic of comprising the above-described first hydrophilic resin. The hydrophilic resin has a characteristic of using at least one of the resins listed above, the resins having a hydrophilic segment comprising a hydrophilic component as a constituent unit and, as described previously, the hydrophilic resin exhibits its insolubility to water and hot water.

The above-described first hydrophilic resin having a hydrophilic segment is obtained by reacting, for example, an organic polyisocyanate with a compound having a high molecular weight hydrophilic polyol and/or polyamine being a hydrophilic component. Hereinafter, compounds used for synthesizing the first hydrophilic resin will be described.

As a hydrophilic component used in the synthesis of the first hydrophilic resin, for example, a high molecular weight hydrophilic polyol and/or a polyamine having, at a terminal thereof, a hydrophilic group such as a hydroxyl group, an amino group, and a carboxyl group and having a weight average molecular weight (a value in terms of standard polystyrene measured by GPC) in a range of 400 to 8,000 are preferable. More specifically, the hydrophilic component is, for example, a hydrophilic polyol having a hydroxyl group at a terminal thereof, and examples thereof include polyethylene glycol, polyethylene glycol/polytetramethylene glycol copolymers, polyethylene glycol/polypropylene glycol copolymers, polyethylene glycol adipate polyol, polyethylene glycol succinate polyol, polyethylene glycol/poly  $\epsilon$ -lactone copolymers, polyethylene glycol/polyvalero lactone copolymers.

Moreover, the hydrophilic component used in the synthesis of the first hydrophilic resin is a hydrophilic polyamine having an amino group at a terminal thereof, and examples thereof include polyethylene oxide diamine, polyethylene oxide-propylene oxide diamine, polyethylene oxide triamine, and polyethylene oxide-propylene oxide triamine. Other hydrophilic components include ethylene oxide adducts having a carboxyl group or a vinyl group.

The first hydrophilic resin can also be synthesized by using another polyol, polyamine, polycarboxylic acid, or the like not having a hydrophilic chain together with the above-described hydrophilic component for the purpose of imparting water resistance to the first hydrophilic resin.

The organic polyisocyanate used in the synthesis of the first hydrophilic resin is not particularly limited, and any of publicly known organic polyisocyanates used in the conventional synthesis of polyurethane resins can be used. As a preferable organic polyisocyanate, for example, 4,4'-diphenylmethane-diisocyanate (hereinafter, abbreviated as MDI), dicyclohexylmethane-4,4'-diisocyanate (hereinafter, abbreviated as hydrogenated MDI), isophorone diisocyanate, 1,3-xylylene diisocyanate, 1,4-xylylene diisocyanate, 2,4-tolylene diisocyanate, m-phenylene diisocyanate, p-phenylene diisocyanate, and so on can be used, or a polyurethane prepolymer or the like obtained by reacting the above organic polyisocyanate with a low molecular weight polyol or polyamine so as to form a terminal isocyanate can also be used.

Moreover, as a chain extender used in synthesizing the first hydrophilic resin as necessary, any of the publicly known conventional chain extenders such as, for example, a low molecular weight diol and diamine can be used without particular limitation. Specific examples of the chain extender include ethylene glycol, 1,3-propanediol, 1,4-butanediol, 1,5-pentanediol, ethylenediamine, and hexamethylenediamine.

It is preferable that the first hydrophilic resin having a hydrophilic segment in the molecular chain, the first hydrophilic resin obtained by allowing the above described raw material components to react, has a weight average molecular weight (a value in terms of standard polystyrene measured by GPC, the same applies hereinafter) in a range of 3,000 to 800,000. More preferable weight average molecular weight is in a range of 5,000 to 500,000.

It is preferable that the content of the hydrophilic segment in the particularly suitable first hydrophilic resin that can be utilized for the method for removing radioactive cesium of the first present invention is in a range of 20 to 80 mass %, more preferably in a range of 30 to 70 mass %. It is not preferable that a resin having a hydrophilic segment content of less than 20 mass % is used because the hydrophilic resin tends to be inferior in water-absorbing performance and the radioactive cesium removing property tends to be deteriorated. On the other hand, it is not preferable that the resin having a hydrophilic segment content exceeding 80 mass % is used because the hydrophilic resin becomes inferior in water resistance.

#### (Second Hydrophilic Resin)

The hydrophilic resin that characterizes the second present invention (hereinafter, referred to as the second hydrophilic resin) comprises at least one selected from the group consisting of a hydrophilic polyurethane resin, a hydrophilic polyurea resin, and a hydrophilic polyurethane-polyurea resin each having a hydrophilic segment comprising a hydrophilic component as a constituent unit and further each having, in the main chain and/or a side chain in the structure thereof, a polysiloxane segment. Each of these segments is randomly bonded through a urethane bond, a urea bond, a urethane-urea bond, or the like in the case where a chain extender is not used at the time of synthesizing the second hydrophilic resin. In the case where a chain extender is used at the time of synthesizing the second hydrophilic resin, the structure is made so that a

short chain that is a residue of the chain extender is present, together with the above-described bonds, between the above-described bonds.

The second hydrophilic resin has a hydrophilic segment in the structure thereof in the same way as in the case of the previously described first hydrophilic resin and, in addition to this, further has a polysiloxane segment in the structure thereof. By constituting the second hydrophilic resin as described here, more useful effect that the water resistance and the blocking resistance performance (sticking resistance) of the surface are improved can be obtained and it becomes possible to achieve the above-described intended purpose of the second present invention more favorably in the case where the resin is used in a form such as a resin film or sheet. Here, the polysiloxane segment introduced in the resin molecule is fundamentally hydrophobic (water-repellent), however in the case where the polysiloxane segment is introduced in the resin structure by an amount of a particular range, the resin is known to become a resin having "environmental responsiveness" (KOBUNSHI RONBUNSHU vol. 48, no. 4, p. 227 (1991)). "Environmental responsiveness" in a resin as described in the literature is a phenomenon that the surface of the resin is completely covered by the polysiloxane segment in a dry state, however, in the state in which the resin is immersed in water, the polysiloxane segment is buried in the resin.

In the second present invention, the phenomenon of the "environmental responsiveness" exhibited by the resin by introducing a polysiloxane segment in the structure of the resin to be used is utilized for the removing processing of radioactive cesium, and thereby the processing is made more effective. The second hydrophilic resin used in the present invention exhibits excellent water absorbency due to the hydrophilic segment present in the structure thereof in the same way as in the case of the aforementioned first hydrophilic resin, can quickly take in ionized radioactive cesium, and is effective for the removing processing of the ionized radioactive cesium. However, according to the studies of the present inventors, there has been a problem as described below in putting a hydrophilic resin into practical use in the case where the structural characteristic of the resin to be used is only to have a hydrophilic segment in the structure thereof. Namely, it becomes necessary in applying the removing processing to radioactive cesium to, for example, make a resin composition to be used in a form such as a sheet form by applying a base material with the resin composition and a film form and to immerse the sheet or the film in the waste liquid containing radioactive cesium, or to make the sheet or the film as a cover for the solid matter containing radioactive cesium. In such cases, durability to the above-described removing processing of radioactive cesium is required for the resin film or the like to be used. However, in the case where the resin having such a structure as the aforementioned first hydrophilic resin has, it is hard to say that the durability is sufficient depending on the use state. The present inventors have made diligent studies against the problem and, as a result thereof, have found that the water resistance and the blocking resistance performance (sticking resistance) of the surface can be improved by further introducing a polysiloxane segment in the molecule (in the structure) of the hydrophilic resin to be used. Namely, the resin constitution becomes a resin constitution by which the resin film or the like exhibits a sufficient water resistant function and the like and more effective removing processing of radioactive cesium can be applied

even in the case of the above-described use form by making the structure of resin so as to be a structure such as the second hydrophilic resin.

It is considered that, in the second present invention, the second hydrophilic resin composition in which a zeolite is dispersed together with the second hydrophilic resin exhibiting the above-described excellent function is used for the removing processing of radioactive cesium and therefore the radioactive cesium has been fixed by the dispersed zeolite more quickly and effectively and immobilized by the resin from the aforementioned reason.

Next, the description will be made with regard to a raw material for forming the second hydrophilic resin that can realize the above-described excellent performance. A preferable second hydrophilic resin is a hydrophilic resin having a hydrophilic segment in the structure thereof, having, in the main chain and/or a side chain in the structure thereof, a polysiloxane segment, and obtained by reacting an organic polyisocyanate, a high molecular weight hydrophilic polyol and/or polyamine being a hydrophilic component, and a compound having at least one active hydrogen-containing group and a polysiloxane segment in the same molecule. Specifically, the preferable second hydrophilic resin is a hydrophilic resin comprising at least one selected from the group consisting of a hydrophilic polyurethane resin, hydrophilic polyurea resin, and a hydrophilic polyurethane-polyurea resin each having a polysiloxane segment. As described here, the second hydrophilic resin is obtained from, as a part of a raw material, the compound having at least one active hydrogen-containing group and a polysiloxane segment in the same molecule, and examples of a specific polysiloxane compound used in synthesizing the second hydrophilic resin, the specific polysiloxane compound usable for introducing a polysiloxane segment in the second hydrophilic resin molecule include polysiloxane compounds having one or two or more reactive groups

specifically such as an amino group, an epoxy group, a hydroxyl group, a mercapto group, and a carboxyl group in the molecule. Preferable examples of the polysiloxane compound having the above-described reactive groups include the following compounds. In addition, a lower alkylene group in the following compounds means a lower alkylene group having about 1 to about 8 carbon atoms.

#### Amino-Modified Polysiloxane Compounds



#### Epoxy-Modified Polysiloxane Compounds



## 17

## Alcohol-Modified Polysiloxane Compounds



## Mercapto-Modified Polysiloxane Compounds



## Carboxyl-Modified Polysiloxane Compounds



## 18



(a = 1~300, b = 2~200, R = a lower alkylene group)



(m = 1~300, R = a lower alkylene group)

15. Among the polysiloxane compounds having an active hydrogen-containing group as described above, polysiloxane polyols and polysiloxane polyamines are particularly useful. In addition, any of the listed compounds is a preferable compound used in the second present invention, however the present invention is not limited to these exemplified compounds. Accordingly, not only above-described exemplified compounds but also any of other compounds currently sold and readily available from the market, the compounds having the similar constitution can be used in the second present invention.

As described previously, it is preferable to use a high molecular weight hydrophilic polyol and/or polyamine being a hydrophilic component in the synthesis of the second hydrophilic resin having a hydrophilic segment. A hydrophilic compound having a hydroxyl group, an amino group, a carboxyl group, or the like and having a weight average molecular weight in a range of 400 to 8,000 is preferable as such a hydrophilic component. The preferable specific examples of 30 the hydrophilic component are the same as the preferable specific examples described previously in the first hydrophilic resin, and therefore the description is omitted. Moreover, the organic polyisocyanates and chain extenders described in the description of the first hydrophilic resin can 35 also be used in addition to the hydrophilic component in synthesizing the second hydrophilic resin.

Another polyol, polyamine, polycarboxylic acid, and so on not having a hydrophilic chain can be used together with the above-described hydrophilic component in the same way as 40 in the case of the first hydrophilic resin for the purpose of imparting water resistance to the second hydrophilic resin.

It is preferable that the second hydrophilic resin having a hydrophilic segment and a polysiloxane segment in the molecular chain, the second hydrophilic resin obtained using 45 the above-described raw material components, has a weight average molecular weight (in terms of standard polystyrene measured by GPC) in a range of 3,000 to 800,000. More preferable weight average molecular weight is in a range of 5,000 to 500,000.

50. It is preferable that the content of the polysiloxane segment in the second hydrophilic resin particularly suitable for using in the second present invention is in a range of 0.1 to 12 mass %, particularly preferably in a range of 0.5 to 10 mass %. It is not preferable that the content of the polysiloxane segment is 55 less than 0.1 mass % because the exhibition of the water resistance and the blocking resistance of the surface that is the intended purpose of the present invention becomes insufficient, and, on the other hand, it is not preferable that the content of the polysiloxane segment exceeds 12 mass % 60 because the water repellency due to the polysiloxane segment becomes strong resulting in deterioration of the water-absorbing performance.

Moreover, it is preferable that the content of the hydrophilic segment in the second hydrophilic resin particularly suitable for using in the second present invention is in a range of 20 to 80 mass %, further more preferably in a range of 30 to 70 mass %. It is not preferable that the content of the hydrophilic segment is less than 20 mass % because the water-absorbing performance tends to be deteriorated. On the other hand, it is not preferable that the content of the hydrophilic segment exceeds 80 mass % because the second hydrophilic resin becomes inferior in water resistance.

Hereinafter, the description will be made with regard to each hydrophilic resin used in the third or the fourth present invention, however in the third or the fourth present invention, there is a difference when compared with the above-described first or second present invention in that not only radioactive cesium present in a radioactive waste liquid or a radioactive solid matter but also both of radioactive iodine and radioactive cesium can be removed.

(Third Hydrophilic Resin)

The hydrophilic resin that characterizes the third present invention (hereinafter, referred to as the third hydrophilic resin) has a characteristic of having: a hydrophilic segment comprising a hydrophilic component as a constituent unit; and at least one tertiary amino group. The third hydrophilic resin may be a hydrophilic resin having: a hydrophilic segment comprising a hydrophilic component as a constituent unit; and at least one tertiary amino group; in the structure thereof. Each of these segments is randomly bonded through a urethane bond, a urea bond, a urethane-urea bond, or the like in the case where a chain extender is not used at the time of synthesizing the third hydrophilic resin. In the case where a chain extender is used at the time of synthesizing the third hydrophilic resin, the structure is made so that a short chain that is a residue of the chain extender is present, together with the above-described bonds, between the above-described bonds.

The third hydrophilic resin composition that can be utilized for the method for removing radioactive iodine and radioactive cesium in the third present invention (hereinafter, referred to as the third hydrophilic resin composition) comprises the third hydrophilic resin and a zeolite, and it becomes possible to apply removing processing to both of radioactive iodine and radioactive cesium together by using the composition. The present inventors consider as follows with regard to the reason why such processing becomes possible. First of all, the third hydrophilic resin exhibits excellent water absorbency due to the hydrophilic segment in the structure thereof, and with regard to exhibiting excellent water absorbency, the third hydrophilic resin is similar to the hydrophilic resins that constitute the first or the second present invention the object of which is to remove radioactive cesium. Therefore, the effect on the removal of radioactive cesium similar to the effect of the first or the second present invention can be obtained also in the third present invention using the third hydrophilic resin.

In the third hydrophilic resin, a tertiary amino group is further introduced in the main chain and/or a side chain in the structure thereof, thereby an ion bond is formed between ionized radioactive iodine and the tertiary amino group, and, as a result thereof, radioactive iodine is considered to be fixed in the third hydrophilic resin in addition to the effect on the above-described removal of radioactive cesium. However, since the above-described ion bond easily dissociates under the presence of moisture, the fixed radioactive iodine is con-

sidered to be discharged again from the resin after a certain period of time is passed, and the present inventors have anticipated that it is difficult to remove radioactive iodine in a state in which the fixing state of radioactive iodine within the resin is immobilized even though the resin having the above-described constitution is used. However, as a result of studies by the present inventors, it has been found that the ionically bonded radioactive iodine, in fact, remains to be fixed within the resin after a long period of time is passed. The reason is uncertain, however the present inventors consider as follows. Namely, the present inventors estimate that, in the third hydrophilic resin used in the present invention, a hydrophobic part is also present in the molecule and the hydrophobic part surrounds, after the ion bond is formed between the tertiary amino group in the resin and radioactive iodine, the circumferences of the hydrophilic part (the hydrophilic segment) and the ion bond. It is considered from the reason as described here that radioactive iodine can be immobilized within the resin and the removal of radioactive iodine becomes possible by using the third hydrophilic resin composition comprising the third hydrophilic resin having a particular structure in the present invention.

Furthermore, as described in detail previously in the description of the first present invention and the second present invention, the third hydrophilic resin composition also comprises third hydrophilic resin having a hydrophilic segment and a zeolite, therefore the removing processing of radioactive cesium in addition to the above-described removal of radioactive iodine also becomes possible, and, as a result thereof, it is considered that applying removal processing to both of radioactive iodine and radioactive cesium together has been achieved by the third present invention.

The third hydrophilic resin composition comprises the third hydrophilic resin, and the hydrophilic resin has a characteristic of having: a hydrophilic segment comprising a hydrophilic component as a constituent unit; and at least one tertiary amino group. Specific examples of the third hydrophilic resin include at least one selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a tertiary amino group.

Such a hydrophilic resin is obtained by reacting an organic polyisocyanate, a high molecular weight hydrophilic polyol and/or polyamine being a hydrophilic component, and a compound having at least one active hydrogen-containing group and at least one tertiary amino group in the same molecule. Namely, examples of a compound used for introducing a hydrophilic segment and a tertiary amino group in the structure of the third hydrophilic resin include a compound having at least one active hydrogen-containing group (reactive group) in the molecule and having, in the molecular chain, a tertiary amino group. Examples of the compound having at least one active hydrogen-containing group include a compound having a reactive group such as an amino group, an epoxy group, a hydroxyl group, a mercapto group, an acid halide group, a carboxyester group, and an acid anhydride group.

Preferable examples of the above-described tertiary amino group-containing compound having a reactive group include compounds represented by the following general formulas (2) to (4).



[In the formula (2),  $R_1$  represents an alkyl group having 20 or less carbon atoms, an alicyclic group, or an aromatic group (which may be substituted with a halogen or an alkyl group),  $R_2$  and  $R_3$  respectively represent an lower alkylene group (having about 1 to about 8 carbon atoms) which may be linked through  $—O—$ ,  $—CO—$ ,  $—COO—$ ,  $—NHCO—$ ,  $—S—$ ,  $—SO—$ ,  $—SO_2—$ , or the like, X and Y represent a reactive group such as  $—OH$ ,  $—COOH$ ,  $—NH_2$ ,  $—NHR_1$  (the definition of  $R_1$  is the same definition as described above), or  $—SH$ , and X and Y may be the same or different; moreover, X and Y may be an epoxy group, an alkoxy group, an acid halide group, an acid anhydride group, or a carboxyester group capable of deriving the above reactive group.]



[In the formula (3), the definition of  $R_1$ ,  $R_2$ ,  $R_3$ ,  $X$ , and  $Y$  is the same definition as in the above formula (2), however the two  $R_1$  may form a cyclic structure;  $R_4$  represents  $-(CH_2)_n-$  ( $n$  is an integer of 0 to 20).]



[In the formula (4), the definition of X and Y is the same definition as in the above formula (2), W represents a nitrogen-containing heterocyclic ring, a nitrogen- and oxygen-containing heterocyclic ring, or a nitrogen- and sulfur-containing heterocyclic ring.]

Specific examples of the compounds represented by the above general formula (2), (3), and (4) include the following compounds. The compounds include N,N-dihydroxyethyl-methylamine, N,N-dihydroxyethyl-ethylamine, N,N-dihydroxyethyl-isopropylamine, N,N-dihydroxyethyl-n-butylamine, N,N-dihydroxyethyl-t-butylamine, methyliminobis-propylamine, N,N-dihydroxyethylaniline, N,N-dihydroxyethyl-m-toluidine, N,N-dihydroxyethyl-p-toluidine, N,N-dihydroxyethyl-m-chloroaniline, N,N-dihydroxyethylbenzylamine, N,N-dimethyl-N',N'-dihydroxyethyl-1,3-diaminopropane, N,N-diethyl-N',N'-dihydroxyethyl-1,3-diaminopropane, N-hydroxyethyl-piperazine, N,N-dihydroxyethyl-piperazine, N-hydroxyethoxyethyl-piperazine, 1,4-bisaminopropyl-piperazine, N-aminopropyl-piperazine, dipicolinic acid, 2,3-diaminopyridine, 2,5-diaminopyridine, 2,6-diamino-4-methylpyridine, 2,6-dihydroxypyridine, 2,6-pyridine-dimethanol, 2-(4-pyridyl)-4,6-dihydroxypyrimidine, 2,6-diaminotriazine, 2,5-diaminotriazole, and 2,5-diaminooxazole.

Moreover, an ethylene oxide adduct, a propylene oxide adduct, or the like of the above tertiary amino compounds may also be used in the present invention. Examples of the adduct include compounds represented by the following structural formula. In addition, m in the following formulas represents an integer of 1 to 60, and n represents an integer of 1 to 6.



As the organic polyisocyanate used in the synthesis of the third hydrophilic resin, the organic polyisocyanates as listed in the description of the first hydrophilic resin can be used.

Moreover, as the hydrophilic component used together with the above-described organic polyisocyanate in the synthesis of the hydrophilic resin that characterizes the present invention, a hydrophilic compound having a hydroxyl group, an amino group, a carboxyl group, or the like and having a weight average molecular weight in a range of 400 to 8,000 is preferable. The preferable specific examples of the hydrophilic component are the same as the preferable specific examples described previously in the description of the first hydrophilic resin, and therefore the description is omitted.

Another polyol, polyamine, polycarboxylic acid, or the like not having a hydrophilic chain can be used together with the above-described hydrophilic component in the same way as in the case of the first hydrophilic resin for the purpose of imparting water resistance to the third hydrophilic resin. Moreover, as the chain extender used in synthesizing the third hydrophilic resin as necessary, any of the chain extenders described previously in the description of the first hydrophilic resin can be used.

It is preferable that the third hydrophilic resin obtained using the above-described raw material components, the third hydrophilic resin having a hydrophilic segment and having, in the molecular chain, a tertiary amino group, has a weight average molecular weight (in terms of polystyrene measured by GPC) in a range of 3,000 to 800,000. Further more preferable weight average molecular weight is in a range of 5,000 to 500,000.

As the particularly suitable third hydrophilic resin used for the method for removing radioactive iodine and radioactive cesium of the third present invention, it is preferable that the content of the tertiary amino group in the resin is 0.1 to 50 eq (equivalent)/kg, further more preferably 0.5 to 20 eq/kg. It is not preferable that the content of the tertiary amino group is less than 0.1 eq/kg, namely less than 1 amino groups per 10,000 molecular weight, because the exhibition of the radioactive iodine removing property that is the intended purpose of the third present invention becomes insufficient. On the other hand, it is not preferable that the content of the tertiary amino group exceeds 50 eq/kg, namely exceeding 500 amino groups per 10,000 molecular weight, because the hydrophobicity becomes strong due to reduction of the hydrophilic part.

in the resin and the third hydrophilic resin becomes inferior in water-absorbing performance.

Moreover, it is preferable that the content of the hydrophilic segment in the particularly suitable third hydrophilic segment in the case where the third hydrophilic resin is used in the third present invention is in a range of 30 to 80 mass %, further more preferably in a range of 50 to 75 mass %. It is not preferable that the content of the hydrophilic segment is less than 30 mass % because the third hydrophilic resin becomes inferior in water-absorbing performance and the radioactive iodine removing property becomes deteriorated. On the other hand, it is not preferable that the content of the hydrophilic segment exceeds 80 mass % because the third hydrophilic resin becomes inferior in water resistance.

(Fourth Hydrophilic Resin)

Hereinafter, the description will be made with regard to the hydrophilic resin used in the fourth present invention. Also in the fourth present invention, both of radioactive iodine and radioactive cesium present in a radioactive waste liquid or a radioactive solid matter can be removed together by using a hydrophilic resin having a particular structure together with a zeolite in the same way as in the above-described third present invention. Furthermore, the hydrophilic resin used in the fourth present invention exhibits a sufficient water resistant function in the same way as in the case of the second hydrophilic resin described previously, and the practicability becomes further improved compared with the practicability of the third present invention by using the hydrophilic resin used in the fourth present invention.

The hydrophilic resin that characterizes the fourth present invention (hereinafter, referred to as the fourth hydrophilic resin) has a characteristic of having a hydrophilic segment comprising a hydrophilic component as a constituent unit and having, in the main chain and/or a side chain in the structure thereof, at least one tertiary amino group and a polysiloxane segment. Namely, the fourth hydrophilic resin may be a hydrophilic resin having: a hydrophilic segment comprising a hydrophilic component as a constituent unit; at least one tertiary amino group; and a polysiloxane segment; in the structure thereof. Each of these segments is randomly bonded through a urethane bond, a urea bond, a urethane-urea bond, or the like in the case where a chain extender is not used at the time of synthesizing the fourth hydrophilic resin. Moreover, in the case where a chain extender is used at the time of synthesizing the fourth hydrophilic resin, the structure is made so that a short chain that is a residue of the chain extender is present, together with the above-described bonds, between the above-described bonds.

The fourth hydrophilic resin composition that can be utilized for the method for removing radioactive iodine and radioactive cesium in the fourth present invention (hereinafter, referred to as the fourth hydrophilic resin composition) comprises the fourth hydrophilic resin having a hydrophilic segment and a tertiary amino group in the structure thereof and a zeolite in the same way as in the case of the third hydrophilic resin. Therefore, it becomes possible to apply removing processing to both of radioactive iodine and radioactive cesium together by using the fourth hydrophilic resin composition in the same way as in the case of using the third hydrophilic resin composition comprising the third hydrophilic resin. The detailed reason is similar to the reason described previously in the case of the third hydrophilic resin composition, and therefore the description is omitted.

The fourth hydrophilic resin is required to be a hydrophilic resin having a polysiloxane segment in the structure thereof in addition to the above-described requirement. Here, as described in the description of the second hydrophilic resin,

the polysiloxane segment introduced in the resin molecule is fundamentally hydrophobic (water-repellent), however in the case where the polysiloxane segment is introduced in the resin structure by an amount of a particular range, the resin is known to become a resin having "environmental responsiveness" (KOBUNSHI RONBUNSHU vol. 48, no. 4, p. 227 (1991)).

The fourth present invention utilizes the phenomenon of the "environmental responsiveness" exhibited by the resin by introducing a polysiloxane segment for the removing processing of radioactive iodine. As described previously, when an ion bond is formed between the tertiary amino group introduced in the hydrophilic resin used in the present invention and radioactive iodine that is an object of processing, the hydrophilicity of the resin is further increased, and thereby, conversely, there is a risk that a problem as described below occurs. Namely, since the removing processing is applied immobilizing radioactive iodine and radioactive cesium as described later in the method for removing radioactive iodine and radioactive cesium of the third present invention, it is preferable that the third hydrophilic resin is used as a form of, for example, a film form or the like, however, in the case, when the amount of the radioactive iodine to be processed is too large, there is a risk that the radioactive iodine poses an obstacle for the water resistance required for the resin. Against this risk, the resin constitution by which the resin to be used exhibits a sufficient water resistant function and more effective removing processing can be applied is realized even in the above-described case by further introducing a polysiloxane segment in the molecule (in the structure) of the hydrophilic resin to be used in the fourth present invention. Namely, the fourth hydrophilic resin can be made more useful when used in the removing processing of radioactive iodine as a result of realizing the water resistance of the resin and the blocking resistance performance (sticking resistance) of the surface by introducing a polysiloxane segment in addition to the water-absorbing performance due to the hydrophilic segment introduced in the structure thereof and the fixing performance to radioactive iodine due to the tertiary amino group.

Furthermore, in the fourth present invention, as described in the first present invention to the third present invention, the removing processing of radioactive cesium in addition to the above-described removal of radioactive iodine is also made possible by using the fourth hydrophilic resin composition comprising a zeolite, and thereby the processing of radioactive iodine and radioactive cesium together is achieved.

Next, the description will be made with regard to a raw material for forming the fourth hydrophilic resin that realizes the above-described performance. The fourth hydrophilic resin has a characteristic of having a hydrophilic segment, a tertiary amino group, and a polysiloxane segment in the structure thereof. Therefore, it is preferable to use, as a part of a raw material, a polyol having at least one tertiary amino group or a polyamine having at least one tertiary amino group, and a compound having at least one active hydrogen-containing group and a polysiloxane segment in the same molecule for the purpose of obtaining the hydrophilic resin. It is preferable to use a tertiary amino group-containing compound as listed below as a compound for introducing the tertiary amino group in the fourth hydrophilic resin. Namely, a compound having at least one active hydrogen-containing group (hereinafter, sometimes described as a reactive group) such as, for example, an amino group, an epoxy group, a hydroxyl group, a mercapto group, an acid halide group, a carboxyester group, and an acid anhydride group in the molecule and having, in the molecular chain, a tertiary amino group is used. Prefer-

able specific examples of the tertiary amino group-containing compound having a reactive group as described above are the same as the specific preferable examples described in the description of the third hydrophilic resin, and therefore the description is omitted.

Moreover, the fourth hydrophilic resin has a characteristic of having a polysiloxane segment in the structure thereof. Examples of the polysiloxane compound usable for introducing a polysiloxane segment in the fourth hydrophilic resin molecule include a compound having one or two or more of reactive groups such as, for example, an amino group, an epoxy group, a hydroxyl group, a mercapto group, and a carboxyl group in the molecule. Preferable examples of the polysiloxane compound having the reactive groups as described above are the same as the preferable examples described in the description of the second hydrophilic resin, and therefore the description is omitted.

Another polyol, polyamine, polycarboxylic acid, or the like not having a hydrophilic chain can be used together with the above-described hydrophilic component in the same way as in the case of the first hydrophilic resin for the purpose of imparting water resistance to the fourth hydrophilic resin. Moreover, as the chain extender used in synthesizing the fourth hydrophilic resin as necessary, the chain extenders described previously in the description of the first hydrophilic resin can be used.

It is preferable that the fourth hydrophilic resin obtained using the above-described raw material components, the fourth hydrophilic resin having a hydrophilic segment and having, in the molecular chain, a tertiary amino group and a polysiloxane segment, has a weight average molecular weight (in terms of standard polystyrene measured by GPC) in a range of 3,000 to 800,000. Further more preferable weight average molecular weight is in a range of 5,000 to 500,000.

It is preferable that the content of the tertiary amino group in the particularly suitable fourth hydrophilic resin used for the method for removing radioactive iodine and radioactive cesium of the fourth present invention is in a range of 0.1 to 50 eq (equivalent)/kg, further more preferably 0.5 to 20 eq/kg. It is not preferable that the content of the tertiary amino group is less than 0.1 eq/kg, namely less than 1 amino groups per 10,000 molecular weight, because the exhibition of the radioactive iodine removing property that is the intended purpose of the fourth present invention, becomes insufficient, and, on the other hand, it is not preferable that the content of the tertiary amino group exceeds 50 eq/kg, namely exceeding 500 amino groups per 10,000 molecular weight, because the hydrophobicity becomes strong due to reduction of the hydrophilic part in the resin and the fourth hydrophilic resin becomes inferior in water-absorbing performance.

Moreover, the content of the polysiloxane segment in the resin as the particularly suitable fourth hydrophilic resin used for the method for removing radioactive iodine and radioactive cesium of the fourth present invention is in a range of 0.1 to 12 mass %, particularly preferably 0.5 to 10 mass %. It is not preferable that the content of the polysiloxane segment is less than 0.1 mass % because the exhibition of the water resistance and the blocking resistance of the surface that is the intended purpose of the present invention becomes insufficient, and, on the other hand, it is not preferable that the content of the polysiloxane segment exceeds 12 mass % because water repellency due to the polysiloxane segment becomes strong, the water-absorbing performance is deteriorated, and the radioactive iodine removing property is inhibited.

Moreover, it is preferable that the content of the hydrophilic segment in the particularly suitable fourth hydrophilic resin in the case where the fourth hydrophilic resin is used in the fourth present invention is in a range of 20 to 80 mass %, further more preferably in a range of 30 to 70 mass %. When the content of the hydrophilic segment is less than 20 mass %, the water-absorbing performance of the fourth hydrophilic resin is deteriorated and the radioactive iodine removing property becomes insufficient. On the other hand, it is not preferable that the content of the hydrophilic segment exceeds 80 mass % because the fourth hydrophilic resin becomes inferior in water resistance.

(Method for Producing Hydrophilic Resin Composition)

The hydrophilic resin composition that is suitable for the method for removing radioactive cesium in the first or the second present invention and the method for removing radioactive iodine and radioactive cesium in the third or the fourth present invention is obtained by dispersing a zeolite in any one of the above-described hydrophilic resins of the first present invention to the fourth present invention. Specifically, the hydrophilic resin composition can be produced by putting a zeolite and a dispersion solvent into any one of the first to the fourth hydrophilic resins as described above and carrying out dispersion operation by a prescribed disperser. As the disperser used for the dispersion, any disperser usually used for pigment dispersion can be used without any problem. Examples of the disperser include a paint conditioner (manufactured by Red Devil, Inc.), a ball mill, a pearl mill (both manufactured by Eirich GmbH), a sand mill, a visco mill, an atlier mill, a basket mill, a wet jet mill (all manufactured by Genus Corporation), however it is preferable to select the disperser taking dispersion performance and economy into consideration. Moreover, as a dispersion medium, a glass bead, a zirconia bead, an alumina bead, a magnetic bead, a stainless steel bead, or the like can be used.

In any of the first invention to the fourth invention, the hydrophilic resin composition in which 1 to 200 mass parts of a zeolite relative to 100 mass parts of the hydrophilic resin is blended as a dispersion ratio of the zeolite to the hydrophilic resin each constituting the hydrophilic resin composition is used. It is not preferable that the dispersion ratio of the zeolite is less than 1 mass parts because there is a risk that the removal of radioactive cesium becomes insufficient, and it is not preferable that the dispersion ratio of the zeolite exceeds 200 mass parts because mechanical properties of the composition become weak, the composition becomes inferior in water resistance, and there is a risk that the composition cannot maintain the shape thereof in radiation-contaminated water.

In addition, in determining the formulation ratio of the hydrophilic resin to the zeolite in the hydrophilic resin composition of the third present invention or the fourth present invention, it is also necessary to consider the point that ions after ion exchange are solved out from the zeolite to the aqueous solution depending on the aforementioned ion exchange order of the zeolite.

In carrying out the method for removing radioactive cesium of the first or the second present invention and the method for removing radioactive iodine and radioactive cesium of the third or the fourth present invention, it is preferable to use any one of the first to the fourth hydrophilic resin compositions comprising the above-described constitution in the following form. Namely, the hydrophilic resin composition formed in a film form obtained by applying release paper, a release film, or the like with a solution of the hydrophilic resin composition so that a thickness after drying becomes 5 to 100  $\mu\text{m}$ , preferably 10 to 50  $\mu\text{m}$  and drying in a drying

furnace is given as an example. In this case, the hydrophilic composition is used as a film for removing radioactive cesium released from the release paper and the release film at the time of use. Moreover, besides the film form, a resin solution obtained from the raw material described previously may be used by applying various base materials with the resin solution or immersing various base materials in the resin solution. As the base material in this case, a metal, glass, timber, fiber, various plastics, and so on can be used.

By immersing the film made of the first or the second hydrophilic resin composition or the sheet obtained by applying various base materials with the first or the second hydrophilic resin composition on various base materials, the film or the sheet obtained as described above, in a radioactive waste liquid, a waste liquid in which a radioactive solid matter is decontaminated with water in advance, or the like, radioactive cesium present in these liquids can be removed. Moreover, against a radiation-contaminated solid matter or the like, the diffusion of radioactive cesium can be prevented by covering the solid matter or the like with the film or the sheet made of the first or the second hydrophilic resin composition. As described previously, particularly in the case where the second hydrophilic resin composition is used, the second hydrophilic resin composition is more useful in removing radioactive iodine because the water resistance of the film or the like and the blocking resistance performance (sticking resistance) of the surface can be realized.

Moreover, by immersing the film made of the third or the fourth hydrophilic resin composition or the sheet obtained by applying various base materials with the third or the fourth hydrophilic resin composition, the film or the sheet obtained as described above, in a radioactive waste liquid, a waste liquid in which a radioactive solid matter is decontaminated with water in advance, or the like, both of radioactive iodine and radioactive cesium can selectively be removed. Moreover, against a radiation-contaminated solid matter or the like, the diffusion of radioactive iodine and radioactive cesium can be prevented by covering the radiation-contaminated solid matter with the film or the sheet made of the third or the fourth hydrophilic resin composition. As described previously, particularly in the case where the fourth hydrophilic resin is used, the fourth hydrophilic resin composition is more useful in removing radioactive iodine because the water resistance of the film or the like and the blocking resistance performance (sticking resistance) of the surface can be realized.

The film or the sheet made of the first or the second hydrophilic resin composition is insoluble to water and therefore can easily be taken out from the waste liquid after decontamination. Thereby, decontamination can be carried out simply and at low cost without the need for special facilities and electricity in removing radioactive cesium. Furthermore, the effect of volume reduction of radioactive waste can be expected by drying the absorbed moisture and heating the film or the sheet at a temperature of 100 to 170° C. in the case of heating the film made of the first hydrophilic resin composition and 120 to 220° C. in the case of heating the film made of the second hydrophilic resin composition because the resin softens and the contraction of volume occurs.

Moreover, the film or the sheet made of the third or the fourth hydrophilic resin composition is insoluble to water and therefore can easily be taken out from the waste liquid after decontamination. Thereby, decontamination can be carried out simply and at low cost without the need for special facilities and electricity in removing both of radioactive iodine and radioactive cesium. Furthermore, the effect of volume reduction of radioactive waste can be expected by drying the absorbed moisture and heating the film or the sheet at a

temperature of 100 to 170° C. because the resin softens and the contraction of volume occurs.

## EXAMPLES

5

Next, the first present invention to the fourth present invention will be described in more detail giving specific Production Examples, Examples, and Comparative Examples, however the first present invention to the fourth present invention are not limited to these examples. Moreover, "parts" and "%" in the following respective examples are based on mass unless otherwise noted.

### Examples and Comparative Examples Relating to First Present Invention and Second Present Invention

15

#### Production Example 1-1

##### Synthesis of Hydrophilic Polyurethane Resin as First Hydrophilic Resin

20

A reaction vessel equipped with a stirrer, a thermometer, a gas introducing tube, and a reflux cooler was purged with nitrogen, 150 parts of polyethylene glycol (molecular weight 2,040) and 20 parts of 1,4-butanediol were dissolved in a mixed solvent of 150 parts of methyl ethyl ketone (hereinafter, abbreviated as MEK) and 200 parts of dimethylformamide (hereinafter, abbreviated as DMF) in the reaction vessel, and the resultant mixture was stirred well at 60° C. And a solution obtained by dissolving 77 parts of hydrogenated MDI in 50 parts of MEK was slowly dropped into the mixture under stirring. After the completion of the dropping, the resultant mixture was subjected to reaction at 80° C. for 7 hours, thereafter 60 parts of MEK was added to the reaction mixture to obtain a hydrophilic resin solution to be used in Example of the first present invention. The resin solution had a viscosity of 280 dPa·s (25° C.) at a solid content of 35%. Moreover, a hydrophilic resin film formed from the resin solution had a breaking strength of 32.5 MPa, a breaking elongation of 450%, a thermal softening temperature of 115° C., and a weight average molecular weight of 78,000.

35

#### Production Example 1-2

##### Synthesis of Hydrophilic Polyurea Resin as First Hydrophilic Resin

40

In a reaction vessel similar to the reaction vessel used in Production Example 1-1, 150 parts of polyethylene oxide diamine ("JEFFAMINE ED" (product name) manufactured by Huntsman Corporation; molecular weight 2,000) and 18 parts of 1,4-diaminobutane were dissolved in 250 parts of

55 DMF. And a solution obtained by dissolving 73 parts of hydrogenated MDI in 100 parts of DMF was slowly dropped into the resultant mixture to react while the resultant mixture was stirred well at an internal temperature of 20 to 30° C. After the completion of the dropping, the internal temperature

60 was gradually raised, and when the internal temperature reached 50° C., the resultant mixture was subjected to reaction for further 6 hours, thereafter 97 parts of DMF was added to the reaction mixture to obtain a hydrophilic resin solution to be used in Example of the first present invention. The resin solution had a viscosity of 210 dPa·s (25° C.) at a solid content of 35%. Moreover, a hydrophilic resin film formed from the resin solution had a breaking strength of 18.3 MPa, a breaking

65

29

elongation of 310%, a thermal softening temperature of 145° C., and a weight average molecular weight of 67,000.

## Production Example 1-3

## Synthesis of Hydrophilic Polyurethane-Polyurea Resin as First Hydrophilic Resin

In a reaction vessel similar to the reaction vessel used in Production Example 1-1, 150 parts of polyethylene oxide diamine ("JEFFAMINE ED" (product name) manufactured by Huntsman Corporation; molecular weight 2,000) and 15 parts of ethylene glycol were dissolved in 250 parts of DMF. And a solution obtained by dissolving 83 parts of hydrogenated MDI in 100 parts of MEK was slowly dropped into the resultant mixture while the resultant mixture was stirred well at an internal temperature of 20 to 30° C. After the completion of dropping, the resultant mixture was subjected to reaction at 80° C. for 6 hours, thereafter 110 parts of MEK was added to the reaction mixture to obtain a hydrophilic resin solution to be used in Example of the first present invention. The resin solution had a viscosity of 250 dPa·s (25° C.) at a solid content of 35%. Moreover, a hydrophilic resin film formed from the resin solution had a breaking strength of 14.7 MPa, a breaking elongation of 450%, a thermal softening temperature of 121° C., and a weight average molecular weight of 71,000.

## Production Example 2-1

## Synthesis of Hydrophilic Polyurethane Resin Having Polysiloxane Segment as Second Hydrophilic Resin

A reaction vessel equipped with a stirrer, a thermometer, a gas introducing tube, and a reflux cooler was purged with nitrogen, and in the reaction vessel, 8 parts of a polydimethylsiloxanepolyol having the following structure (molecular weight 3,200), 142 parts of polyethylene glycol (molecular weight 2,040), and 8 parts of ethylene glycol were dissolved in a mixed solvent of 150 parts of MEK and 140 parts of DMF. And a solution obtained by dissolving 52 parts of hydrogenated MDI in 50 parts of MEK was slowly dropped into the resultant mixture while the resultant mixture was stirred well at 60° C. After the completion of the dropping, the resultant mixture was subjected to reaction at 80° C. for 6 hours, and thereafter 50 parts of MEK was added to the reaction mixture to obtain a solution of a hydrophilic polyurethane resin having a structure specified in the second present invention.



(a is an integer that gives a molecular weight of 3,200)

The obtained resin solution had a viscosity of 410 dPa·s (25° C.) at a solid content of 35%. Moreover, a hydrophilic resin film formed from the resin solution had a breaking strength of 24.5 MPa, a breaking elongation of 450%, and a thermal softening temperature of 105° C.

## Production Example 2-2

## Synthesis of Hydrophilic Polyurea Resin Having Polysiloxane Segment as Second Hydrophilic Resin

In a reaction vessel similar to the reaction vessel used in Production Example 2-1, 5 parts of a polydimethylsilox-

30

anediamine having the following structure (molecular weight 3,880), 145 parts of polyethylene oxide diamine ("JEFFAMINE ED" (product name) manufactured by Huntsman Corporation; molecular weight 2,000), and 8 parts of propylene diamine were dissolved in 180 parts of DMF. And a solution obtained by dissolving 47 parts of hydrogenated MDI in 100 parts of DMF was slowly dropped into the resultant mixture to react while the resultant mixture was stirred well at an internal temperature of 10 to 20° C. After the completion of the dropping, the internal temperature was gradually raised, and when the temperature reached 50° C., the resultant mixture was subjected to reaction for further 6 hours, and thereafter 100 parts of DMF was added to the reaction mixture to obtain a solution of a hydrophilic polyurea resin having a structure specified in the second present invention.



(c is an integer that gives a molecular weight of 3,880)

The obtained resin solution had a viscosity of 250 dPa·s (25° C.) at a solid content of 35%. Moreover, a film formed from the resin solution had a breaking strength of 27.6 MPa, a breaking elongation of 310%, and a thermal softening temperature of 145° C.

## Production Example 2-3

## Synthesis of Hydrophilic Polyurethane-Polyurea Resin Having Polysiloxane Segment as Second Hydrophilic Resin

In a reaction vessel similar to the reaction vessel used in Production Example 2-2, 145 parts of polyethylene glycol (molecular weight 2,040), and 8 parts of 1,3-butylene glycol were dissolved in a mixed solvent of 74 parts of toluene and 197 parts of MEK. And a solution obtained by dissolving 42 parts of hydrogenated MDI in 100 parts of MEK was slowly dropped into the resultant mixture while the resultant mixture was stirred well at 60° C. After the completion of the dropping, the resultant mixture was subjected to reaction at 80° C. for 6 hours to obtain a solution of a hydrophilic polyurethane-polyurea resin having a structure specified in the second present invention. The obtained resin solution had a viscosity of 200 dPa·s (25° C.) at a solid content of 35%. Moreover, a film formed from the resin solution had a breaking strength of 14.7 MPa, a breaking elongation of 450%, and a thermal softening temperature of 90° C.

## Production Example 4a

## Synthesis of Non-Hydrophilic Polyurethane Resin to be Used in Comparative Example of First Present Invention and Second Present Invention

A reaction vessel similar to the reaction vessel used in Production Example 1-1 was purged with nitrogen, and in the reaction vessel, 150 parts of polybutyleneadipate having an average molecular weight of about 2,000 and 15 parts of 1,4-butanediol were dissolved in 250 parts of DMF. And a

31

solution obtained by dissolving 62 parts of hydrogenated MDI in 100 parts of MEK was slowly dropped into the resultant mixture while the resultant mixture was stirred well at 60° C. After the completion of the dropping, the resultant mixture was subjected to reaction at 80° C. for 6 hours, and thereafter 71 parts of MEK was added to the reaction mixture to obtain a non-hydrophilic resin solution to be used in Comparative Example of the first present invention and the second present invention. The resin solution had a viscosity of 320 dPa·s (25° C.) at a solid content of 351. Moreover, a non-hydrophilic resin film formed from the solution had a breaking strength of 45 MPa, a breaking elongation of 480%, a thermal softening temperature of 110° C., and a weight average molecular weight of 82,000.

Production Example 5a

Synthesis of Non-Hydrophilic  
Polyurethane-Polyurea Resin to be Used in  
Comparative Example of First Present Invention and  
Second Present Invention

A reaction vessel similar to the reaction vessel used in Production Example 1-1 was purged with nitrogen, and in the reaction vessel, 150 parts of polybutyleneadipate having an average molecular weight of about 2,000 and 18 parts of hexamethylenediamine were dissolved in 200 parts of DMF. And a solution obtained by dissolving 60 parts of hydrogenated MDI in 100 parts of MEK was slowly dropped into the resultant mixture while the resultant mixture was stirred well at an internal temperature of 20 to 30° C. After the completion of the dropping, the resultant mixture was subjected to reaction at 80° C. for 6 hours, and thereafter 123 parts of MEK was added to the reaction mixture to obtain a non-hydrophilic resin solution to be used in Comparative Example of the first present invention and the second present invention. The resin solution had a viscosity of 250 dPa·s (25° C.) at a solid content of 35%. Moreover, a non-hydrophilic resin film formed from the resin solution had a breaking strength of 14.7 MPa, a breaking elongation of 450%, a thermal softening temperature of 121° C., and a weight average molecular weight of 68,000.

In Table 1, the property, the weight average molecular weight, and the content of the polysiloxane segment with regard to the respective resins obtained by respective Production Examples are listed together.

32

TABLE 1

| Properties of respective resins obtained<br>by respective Production Examples |                                 |                                    |                                     |
|-------------------------------------------------------------------------------|---------------------------------|------------------------------------|-------------------------------------|
|                                                                               | Hydrophilic/<br>Non-hydrophilic | Weight average<br>molecular weight | Polysiloxane<br>segment content (%) |
| 10                                                                            | Production Example 1-1          | Hydrophilic                        | 78,000                              |
|                                                                               | Production Example 1-2          | Hydrophilic                        | 67,000                              |
|                                                                               | Production Example 1-3          | Hydrophilic                        | 71,000                              |
| 15                                                                            | Production Example 2-1          | Hydrophilic                        | 86,000                              |
|                                                                               | Production Example 2-2          | Hydrophilic                        | 71,000                              |
|                                                                               | Production Example 2-3          | Hydrophilic                        | 65,000                              |
| 20                                                                            | Production Example 4a           | Non-hydrophilic                    | 82,000                              |
|                                                                               | Production Example 5a           | Non-hydrophilic                    | 68,000                              |
|                                                                               |                                 |                                    | Not contained                       |

Examples 1-1 to 1-3 and Comparative Examples 1a to 2a of First Present Invention, and Examples 2-1 to 2-3 and Comparative Examples 1a to 2a of Second Present Invention

35 Dispersion processing was applied for 24 hours by a ball mill with a high density alumina ball (3.5 g/ml) using each of the resin solutions obtained by the above-described Production Examples and a zeolite (manufactured by Sun Zeolite Kogyo K.K.) with each combination (based on mass) shown in Tables 2-1 and 2-2. And the contents after the dispersion were taken out through a 100 mesh sieve made of a polyester resin to obtain each resin composition in a liquid state comprising each resin solution and a zeolite. The resin compositions of Examples and Comparative Examples with regard to 40 the first present invention are shown in Table 2-1 together, and the resin compositions of Examples and Comparative Examples with regard to the second present invention are shown in Table 2-2 together.

45

TABLE 2-1

Preparation of resin compositions of Examples and Comparative Examples with regard to the first present invention [mass parts]

|                                             | Example 1-1 | Example 1-2 | Example 1-3 | Comparative Example 1A | Comparative Example 2A |
|---------------------------------------------|-------------|-------------|-------------|------------------------|------------------------|
| Resin solution of<br>Production Example 1-1 | 100         |             |             |                        |                        |
| Resin solution of<br>Production Example 1-2 |             | 100         |             |                        |                        |
| Resin solution of<br>Production Example 1-3 |             |             | 100         |                        |                        |
| Resin solution of<br>Production Example 4a  |             |             |             | 100                    |                        |
| Resin solution of<br>Production Example 5a  |             |             |             |                        | 100                    |
| Zeolite                                     | 10          | 15          | 20          | 10                     | 20                     |
| Solvent (MEK/DMF = 7/3)                     | 70          | 85          | 100         | 70                     | 100                    |

TABLE 2-2

| Preparation of resin compositions of Examples and Comparative Examples with regard to the second present invention [mass parts] |             |             |             |                        |                        |
|---------------------------------------------------------------------------------------------------------------------------------|-------------|-------------|-------------|------------------------|------------------------|
|                                                                                                                                 | Example 2-1 | Example 2-2 | Example 2-3 | Comparative Example 1a | Comparative Example 2a |
| Resin solution of                                                                                                               | 100         |             |             |                        |                        |
| Production Example 2-1                                                                                                          |             |             |             |                        |                        |
| Resin solution of                                                                                                               |             | 100         |             |                        |                        |
| Production Example 2-2                                                                                                          |             |             |             |                        |                        |
| Resin solution of                                                                                                               |             |             | 100         |                        |                        |
| Production Example 2-3                                                                                                          |             |             |             |                        |                        |
| Resin solution of                                                                                                               |             |             |             | 100                    |                        |
| Production Example 4a                                                                                                           |             |             |             |                        |                        |
| Resin solution of                                                                                                               |             |             |             |                        | 100                    |
| Production Example 5a                                                                                                           |             |             |             |                        |                        |
| Zeolite                                                                                                                         | 15          | 20          | 25          | 15                     | 25                     |
| Solvent (MEK/DMF = 7/3)                                                                                                         | 85          | 100         | 115         | 85                     | 115                    |

[Evaluation of First Present Invention and Second Present Invention]

The following tests were carried out using each resin composition of Examples and Comparative Examples of the second present invention to check the usefulness of each of the obtained resin compositions provided by the second present invention. Release paper was applied with each resin composition having the formulation shown in Table 2-2 and dried by heating at 110° C. for 3 minutes to volatilize the solvent, and each resin film having a thickness of about 20 µm was formed. The following items were evaluated using each resin film thus obtained and formed from each resin composition of Examples 2-1 to 2-3 and Comparative Examples 1a and 2a of the second present invention.

<Blocking Resistance (Sticking Resistance) of Resin Film>

Film faces of each resin film of Examples 2-1 to 2-3 and Comparative Examples 1a and 2a formed from each resin composition were placed face to face, thereafter the films were left at 40° C. for 1 day while a load of 0.29 MPa was applied thereon. After that, the blocking property of the films with the faces placed face to face was visually observed and evaluated according to the following criteria. And the obtained results are shown in Table 3 together.

Good: No blocking property was observed.

Fair: The blocking property was slightly observed.

Poor: The blocking property was observed.

<Water Resistance of Resin Film>

Each resin film formed from each resin composition of Examples 2-1 to 2-3 and Comparative Examples 1a and 2a was cut in a shape having a thickness of 20 µm and a longitudinal length of 5 cm× a transversal length of 1 cm and immersed in water having a temperature of 25° C. for 12 hours, and the water resistance was evaluated by measuring the coefficient of expansion in the longitudinal direction of the immersed film.

In addition, the coefficient of expansion (expansion rate) was calculated by the following method, and the water resistance was evaluated by rating a film having a coefficient of

expansion of 200% or less as "Good" and a film having a coefficient of expansion of more than 200% as "Poor". The obtained results are shown in Table 3 together.

$$\text{Coefficient of expansion (\%)} = (\text{Longitudinal length after test} / \text{Original longitudinal length}) \times 100$$

TABLE 3

| Evaluation results (blocking resistance and water resistance) |                     |                                                 |
|---------------------------------------------------------------|---------------------|-------------------------------------------------|
|                                                               | Blocking resistance | Water resistance (Coefficient of expansion (%)) |
| Example 2-1                                                   | Good                | Good (145)                                      |
| Example 2-2                                                   | Good                | Good (151)                                      |
| Example 2-3                                                   | Good                | Good (168)                                      |
| Comparative Example 1a                                        | Poor                | Good (105)                                      |
| Comparative Example 2a                                        | Poor                | Good (103)                                      |

<Evaluation of Removal of Cesium>

A cesium-removing function of each of the obtained resin compositions provided by the first present invention and the second present invention was checked in the following manner. Using each resin composition of Examples and Comparative Examples of the first present invention and the second present invention, release paper was applied with each resin composition and dried by heating at 110° C. for 3 minutes to volatilize the solvent, and each resin film having a thickness of about 20 µm was formed. The effect on the removal of cesium ion was evaluated by the following method using each resin film of Examples and Comparative Examples of the first present invention and the second present invention thus obtained.

(Preparation of Cesium Solution for Evaluation Test>

A cesium solution for the evaluation test was prepared by dissolving cesium chloride in ion exchanged pure water so that the solution had a cesium ion concentration of 100 mg/L (100 ppm). In addition, when cesium ion can be removed, radioactive cesium can be removed naturally.

35

(Evaluation Results with Regard to Resin Composition of Example 1-1 of First Present Invention)

In 100 ml of the cesium solution prepared previously for the evaluation test and having an ion concentration of 100 ppm, 20 g of the resin film prepared using the hydrophilic resin composition of Example 1-1 was immersed (25° C.), and the cesium ion concentration in the solution was measured by an ion chromatograph (IC2001 manufactured by Tosoh Corporation) every time a predetermined time was elapsed. In Table 4, the removing rate of the cesium ion in the solutions every time a predetermined time was elapsed was listed together with the concentration of the cesium ion.

36

Moreover, the result of the obtained change of the cesium ion concentration with time is shown in FIG. 1.

(Evaluation Results with Regard to Resin Compositions of Examples 1-2 and 1-3 of First Present Invention)

The cesium ion concentrations in the solutions every time a predetermined time was elapsed were measured in the same manner as in Example 1-1 except that 20 g of each resin film prepared by the hydrophilic resin composition of Example 1-2 or Example 1-3 was used for each test. The obtained results are shown in Table 4 and FIG. 1 in the same manner as in Example 1-1 described previously.

TABLE 4

| Evaluation results in the case where the resin composition films of Examples 1-1 to 1-3 of the first present invention were used |                                |                              |                                |                              |                                |                              |                              |
|----------------------------------------------------------------------------------------------------------------------------------|--------------------------------|------------------------------|--------------------------------|------------------------------|--------------------------------|------------------------------|------------------------------|
| Immersion time (Hr)                                                                                                              | Example 1-1                    |                              | Example 1-2                    |                              | Example 1-3                    |                              | Cesium ion removing rate (%) |
|                                                                                                                                  | Cesium ion concentration (ppm) | Cesium ion removing rate (%) | Cesium ion concentration (ppm) | Cesium ion removing rate (%) | Cesium ion concentration (ppm) | Cesium ion removing rate (%) |                              |
| 0                                                                                                                                | 100.0                          | —                            | 100.0                          | —                            | 100.0                          | —                            |                              |
| 1                                                                                                                                | 47.5                           | 52.5                         | 38.1                           | 61.9                         | 33.8                           | 66.2                         |                              |
| 5                                                                                                                                | 18.3                           | 81.7                         | 11.5                           | 88.5                         | 7.8                            | 92.2                         |                              |
| 15                                                                                                                               | 10.7                           | 89.3                         | 5.1                            | 94.9                         | 1.8                            | 98.2                         |                              |
| 24                                                                                                                               | 7.5                            | 92.5                         | 2.3                            | 97.7                         | 0.5                            | 99.5                         |                              |

35 (Evaluation Results with Regard to Resin Compositions of Examples 2-1 to 2-3 of Second Present Invention)

In 100 ml of the cesium solution, 20 g of each hydrophilic resin composition film of Examples 2-1 to 2-3 was immersed (25° C.), and the cesium ion concentration in the solution was measured by an ion chromatograph (IC2001 manufactured by Tosoh Corporation) every time a predetermined time was elapsed. And the removing rate of the cesium ion in the solution was calculated. The results are shown in Table 5 and FIG. 2.

TABLE 5

| Evaluation results in the case where the resin films of Examples 2-1 to 2-3 of the second present invention were used |                                |                              |                                |                              |                                |                              |                              |
|-----------------------------------------------------------------------------------------------------------------------|--------------------------------|------------------------------|--------------------------------|------------------------------|--------------------------------|------------------------------|------------------------------|
| Immersion time (Hr)                                                                                                   | Example 2-1                    |                              | Example 2-2                    |                              | Example 2-3                    |                              | Cesium ion removing rate (%) |
|                                                                                                                       | Cesium ion concentration (ppm) | Cesium ion removing rate (%) | Cesium ion concentration (ppm) | Cesium ion removing rate (%) | Cesium ion concentration (ppm) | Cesium ion removing rate (%) |                              |
| 0                                                                                                                     | 100.0                          | —                            | 100.0                          | —                            | 100.0                          | —                            |                              |
| 1                                                                                                                     | 48.1                           | 51.9                         | 39.4                           | 60.6                         | 34.5                           | 65.5                         |                              |
| 5                                                                                                                     | 19.6                           | 80.4                         | 12.1                           | 87.9                         | 8.3                            | 91.7                         |                              |
| 15                                                                                                                    | 11.5                           | 88.5                         | 6.8                            | 93.2                         | 2.3                            | 97.7                         |                              |
| 24                                                                                                                    | 8.8                            | 91.2                         | 3.5                            | 96.5                         | 1.0                            | 99.0                         |                              |

(Evaluation Results with Regard to Resin Compositions of Comparative Examples 1a and 2a of First Present Invention and Comparative Examples 1a and 2a of Second Present Invention)

The cesium ion concentrations in the solutions were measured every time a predetermined time was elapsed in the same manner as in Example 1-1 except that 20 g of each resin film prepared by the non-hydrophilic resin composition of Comparative Example 1A or 2A, or Comparative Example 1a or 2a was used for each test. The obtained results are shown in Table 6-1, 6-2, and FIG. 3 in the same manner as in the case of Example 1-1 described previously. As clearly understood from these results, the superiority of the cesium ion removing performance in Examples of the first present invention and the second present invention was confirmed.

TABLE 6-1

| Evaluation results in the case where the resin composition films of Comparative Examples of 1A to 2A of the first present invention were used |                                |                              |                                |                              |
|-----------------------------------------------------------------------------------------------------------------------------------------------|--------------------------------|------------------------------|--------------------------------|------------------------------|
|                                                                                                                                               | Comparative Example 1A         |                              | Comparative Example 2A         |                              |
| Immersion time (Hr)                                                                                                                           | Cesium ion concentration (ppm) | Cesium ion removing rate (%) | Cesium ion concentration (ppm) | Cesium ion removing rate (%) |
| 0                                                                                                                                             | 100.0                          | —                            | 100.0                          | —                            |
| 1                                                                                                                                             | 98.7                           | 1.3                          | 97.0                           | 3.0                          |
| 5                                                                                                                                             | 97.3                           | 2.7                          | 96.5                           | 3.5                          |
| 15                                                                                                                                            | 97.0                           | 3.0                          | 95.3                           | 4.7                          |
| 24                                                                                                                                            | 96.8                           | 3.2                          | 94.5                           | 5.5                          |

TABLE 6-2

| Evaluation results in the case where the resin composition films of Comparative Examples of 1a to 2a of the second present invention were used |                                |                              |                                |                              |
|------------------------------------------------------------------------------------------------------------------------------------------------|--------------------------------|------------------------------|--------------------------------|------------------------------|
|                                                                                                                                                | Comparative Example 1a         |                              | Comparative Example 2a         |                              |
| Immersion time (Hr)                                                                                                                            | Cesium ion concentration (ppm) | Cesium ion removing rate (%) | Cesium ion concentration (ppm) | Cesium ion removing rate (%) |
| 0                                                                                                                                              | 100.0                          | —                            | 100.0                          | —                            |
| 1                                                                                                                                              | 99.5                           | 0.5                          | 99.0                           | 1.0                          |
| 5                                                                                                                                              | 98.3                           | 1.7                          | 97.7                           | 2.3                          |
| 15                                                                                                                                             | 97.1                           | 2.9                          | 96.8                           | 3.2                          |
| 24                                                                                                                                             | 96.8                           | 3.2                          | 95.3                           | 4.7                          |

Examples and Comparative Examples Relating to Third Present Invention and Fourth Present Invention

#### Production Example 3-1

#### Synthesis of Tertiary Amino Group-Containing Hydrophilic Polyurethane Resin as Third Hydrophilic Resin

A reaction vessel equipped with a stirrer, a thermometer, a gas introducing tube, and a reflux condenser was purged with nitrogen, 150 parts of polyethylene glycol (molecular weight 2,040), 20 parts of N-methyldiethanolamine, and 5 parts of diethylene glycol were dissolved in a mixed solvent of 200 parts of MEK and 150 parts of DMF in the reaction vessel, and the resultant mixture was stirred well at 60° C. And a solution obtained by dissolving 74 parts of hydrogenated MDI in 112 parts of MEK was slowly dropped into the mix-

ture under stirring. After the completion of the dropping, the resultant mixture was subjected to reaction at 80° C. for 6 hours to obtain a solution of a hydrophilic resin specified in the third present invention. The resin solution had a viscosity of 530 dPa·s (25° C.) at a solid content of 35%. Moreover, a hydrophilic resin film formed from the solution had a breaking strength of 24.5 MPa, a breaking elongation of 450%, and a thermal softening temperature of 115° C.

#### Production Example 3-2

#### Synthesis of Tertiary Amino Group-Containing Hydrophilic Polyurea Resin as Third Hydrophilic Resin

In a reaction vessel similar to the reaction vessel used in Production Example 3-1, 150 parts of polyethylene oxide diamine ("JEFFAMINE ED" (product name) manufactured by Huntsman Corporation; molecular weight 2,000), 30 parts of methyliminobispropylamine, and 4 parts of 1,4-diamino butane were dissolved in 200 parts of DMF, and the resultant mixture was stirred well at an internal temperature of 20 to 30° C. And a solution obtained by dissolving 83 parts of hydrogenated MDI in 100 parts of DMF was slowly dropped into the resultant mixture under stirring to react. After the completion of the dropping, the internal temperature was gradually raised, and when the temperature reached 50° C., the resultant mixture was subjected to reaction for further 6 hours, and thereafter 195 parts of DMF was added to the reaction mixture to obtain a solution of a hydrophilic resin specified in the third present invention. The resin solution had a viscosity of 230 dPa·s (25° C.) at a solid content of 35%. Moreover, a hydrophilic resin film formed from the resin solution had a breaking strength of 27.6 MPa, a breaking elongation of 310%, and a thermal softening temperature of 145° C.

#### Production Example 3-3

#### Synthesis of Tertiary Amino Group-Containing Hydrophilic Polyurethane-Polyurea Resin as Third Hydrophilic Resin

In a reaction vessel similar to the reaction vessel used in Production Example 3-1, 150 parts of polyethylene oxide diamine ("JEFFAMINE ED" (product name) manufactured by Huntsman Corporation; molecular weight 2,000), 30 parts of N,N-dimethyl-N',N'-dihydroxyethyl-1,3-diaminopropane, and 6 parts of triethylene glycol were dissolved in 140 parts of DMF. And a solution obtained by dissolving 70 parts of hydrogenated MDI in 200 parts of MEK was slowly dropped into the resultant mixture while the resultant mixture was stirred well at an internal temperature of 20 to 30° C. After the completion of the dropping, the resultant mixture was subjected to reaction at 80° C. for 6 hours, and thereafter 135 parts of MEK was added to the reaction mixture to obtain a solution of a hydrophilic resin specified in the third present invention. The resin solution had a viscosity of 280 dPa·s (25° C.) at a solid content of 35%. Moreover, a hydrophilic resin film formed from the solution had a breaking strength of 14.7 MPa, a breaking elongation of 450%, and a thermal softening temperature of 107° C.

#### Production Example 4-1

#### Synthesis of Hydrophilic Polyurethane Resin Having Tertiary Amino Group and Polysiloxane Segment as Fourth Hydrophilic Resin

A reaction vessel equipped with a stirrer, a thermometer, a gas introducing tube, and a reflux cooler was purged with

39

nitrogen, and in the reaction vessel, 8 parts of a polydimethylsiloxanepolyol having the following structure (molecular weight 3,200), 142 parts of polyethylene glycol (molecular weight 2,040), 20 parts of N-methyldiethanolamine, and 5 parts of diethylene glycol were dissolved in a mixed solvent of 100 parts of MEK and 200 parts of DMF. And a solution obtained by dissolving 73 parts of hydrogenated MDI in 100 parts of MEK was slowly dropped into the resultant mixture while the resultant mixture was stirred well at 60° C. After the completion of the dropping, the resultant mixture was subjected to reaction at 80° C. for 6 hours, and thereafter 60 parts of MEK was added to the reaction mixture to obtain a solution of a hydrophilic polyurethane resin having a structure specified in the fourth present invention.



(a is an integer that gives a molecular weight of 3,200)

The obtained resin solution had a viscosity of 330 dPa·s (25° C.) at a solid content of 35%. Moreover, a hydrophilic resin film formed from the solution had a breaking strength of 20.5 MPa, a breaking elongation of 400%, and a thermal softening temperature of 103° C.

#### Production Example 4-2

##### Synthesis of Hydrophilic Polyurea Resin Having Tertiary Amino Group and Polysiloxane Segment as Fourth Hydrophilic Resin

In a reaction vessel similar to the reaction vessel used in Production Example 4-1, 5 parts of a polydimethylsiloxane diaminine having the following structure (molecular weight 3,880), 145 parts of polyethylene oxide diamine ("JEFFAMINE ED" (product name) manufactured by Huntsman Corporation; molecular weight 2,000), 25 parts of methylimino-bispropylamine, and 5 parts of 1,4-diaminobutane were dissolved in 250 parts of DMF and the resultant mixture was stirred well at an internal temperature of 20 to 30° C. And a solution obtained by dissolving 75 parts of hydrogenated MDI in 100 parts of DMF was slowly dropped into the resultant mixture under stirring to react. After the completion of the dropping, the internal temperature was gradually raised, and when the temperature reached 50° C., the resultant mixture was subjected to reaction for further 6 hours, and thereafter 124 parts of DMF was added to the reaction mixture to obtain a solution of a hydrophilic polyurea resin having a structure specified in the fourth present invention.



(c is an integer that gives a molecular weight of 3,880)

The obtained resin solution had a viscosity of 315 dPa·s (25° C.) at a solid content of 35%. Moreover, a hydrophilic resin film formed from the resin solution had a breaking

40

strength of 31.3 MPa, a breaking elongation of 370%, and a thermal softening temperature of 147° C.

#### Production Example 4-3

##### Synthesis of Hydrophilic Polyurethane-Polyurea Resin Having Tertiary Amino Group and Polysiloxane Segment as Fourth Hydrophilic Resin

10 In a reaction vessel similar to the reaction vessel used in Production Example 4-1, 5 parts of an ethylene oxide added type polydimethylsiloxane having the following structure (molecular weight 4,500), 145 parts of polyethylene oxide diamine ("JEFFAMINE ED" (trade name) manufactured by 15 Huntsman Corporation; molecular weight 2,000), 30 parts of N,N-dimethyl-N',N'-dihydroxyethyl-1,3-diaminopropane, and 5 parts of 1,4-diaminobutane were dissolved in a mixed solvent of 150 parts of MEK and 150 parts of DMF, and the resultant mixture was stirred well at an internal temperature 20 of 20 to 30° C. And a solution obtained by dissolving 72 parts of hydrogenated MDI in 100 parts of MEK was slowly dropped into the resultant mixture under stirring. After the completion of the dropping, the resultant mixture was subjected to reaction at 80° C. for 6 hours, and after the completion of the reaction, 75 parts of MEK was added to the reaction mixture to obtain a solution of a hydrophilic polyurethane-polyurea resin having a structure specified in the fourth present invention.



(m and n are integers that give a molecular weight of 4,500)

30 The obtained resin solution had a viscosity of 390 dPa·s (25° C.) at a solid content of 35%. Moreover, a hydrophilic 40 resin film formed from the resin solution had a breaking strength of 22.7 MPa, a breaking elongation of 450%, and a thermal softening temperature of 127° C.

#### Production Example 4b

##### Synthesis of Non-Hydrophilic Polyurethane Resin not Containing Tertiary Amino Group and Polysiloxane Segment to be Used in Comparative Example of Third Present Invention and Fourth Present Invention

45 A reaction vessel similar to the reaction vessel used in Production Example 3-1 was purged with nitrogen, and 150 parts of polybutylene adipate having an average molecular 50 weight of about 2,000 and 15 parts of 1,4-butanediol were dissolved in 250 parts of DMF in the reaction vessel. And a solution obtained by dissolving 62 parts of hydrogenated MDI in 171 parts of DMF was slowly dropped into the resultant mixture while the resultant mixture was stirred well at 60° C. After the completion of the dropping, the resultant mixture 55 was subjected to reaction at 80° C. for 6 hours to obtain a resin solution to be used in Comparative Example. The resin solution had a viscosity of 320 dPa·s (25° C.) at a solid content of 35%. A non-hydrophilic resin film obtained from the resin 60 solution had a breaking strength of 45 MPa, a breaking elongation of 480%, and a thermal softening temperature of 110° C.

## Production Example 5b

Synthesis of Tertiary Amino Group-Containing Non-Hydrophilic Polyurethane Resin to be Used in Comparative Example of Third Present Invention and Fourth Present Invention

A reaction vessel similar to the reaction vessel used in Production Example 3-1 was purged with nitrogen, and in the reaction vessel, 150 parts of polybutyleneadipate having an average molecular weight of about 2,000, 20 parts of N-methyl diethanolamine, and 5 parts of diethylene glycol were dissolved in a mixed solvent of 200 parts of MEK and 150 parts of DMF. And a solution obtained by dissolving 74 parts of hydrogenated MDI in 112 parts of MEK was slowly dropped into the resultant mixture while the resultant mixture was stirred well at 60°C. After the completion of the dropping, the resultant mixture was subjected to reaction at 80°C. for 6 hours to obtain a resin solution to be used in Comparative Example. The resin solution had a viscosity of 510 dPa·s (25°C.) at a solid content of 35%. Moreover, a non-hydrophilic resin film formed from the resin solution had a breaking strength of 23.5 MPa, a breaking elongation of 470%, and a thermal softening temperature of 110°C.

In Table 7-1, the properties with regard to the respective resins to be used in Examples of the third present invention obtained by the above-described Production Examples 3-1 to 3-3 and respective resins to be used in Comparative Examples of the third present invention obtained by Production Examples 4b and 5b are listed together. Specifically as the properties, the evaluation of hydrophilicity, the weight average molecular weight, and the content of the tertiary amino group (equivalent) per 1,000 molecular weight are shown.

TABLE 7-1

| Properties of respective resins obtained by respective Production Examples relating to the third present invention |                             |                                 |                                         |
|--------------------------------------------------------------------------------------------------------------------|-----------------------------|---------------------------------|-----------------------------------------|
|                                                                                                                    | Hydrophilic/Non-hydrophilic | Weight average molecular weight | Tertiary amino group equivalent (eq/kg) |
| Production Example 3-1                                                                                             | Hydrophilic                 | 87,000                          | 0.67                                    |
| Production Example 3-2                                                                                             | Hydrophilic                 | 63,000                          | 0.76                                    |
| Production Example 3-3                                                                                             | Hydrophilic                 | 69,000                          | 1.23                                    |
| Production Example 4b                                                                                              | Non-hydrophilic             | 72,000                          | Not contained                           |

## TABLE 7-1-continued

| Properties of respective resins obtained by respective Production Examples relating to the third present invention |                             |                                 |                                         |
|--------------------------------------------------------------------------------------------------------------------|-----------------------------|---------------------------------|-----------------------------------------|
|                                                                                                                    | Hydrophilic/Non-hydrophilic | Weight average molecular weight | Tertiary amino group equivalent (eq/kg) |
| Production Example 5b                                                                                              | Non-hydrophilic             | 84,000                          | 0.68                                    |

In Table 7-2, the properties with regard to the respective resins to be used in Examples of the fourth present invention obtained by the above-described Production Examples 4-1 to 4-3 and respective resins to be used in Comparative Examples of the fourth present invention obtained by Production Examples 4b and 5b are listed together. Specifically, the evaluation of hydrophilicity, the weight average molecular weight, and the content of the tertiary amino group (equivalent) per 1,000 molecular weight are shown.

TABLE 7-2

| Properties of respective resins of respective Production Examples relating to the fourth present invention |                             |                                 |                                         |                                  |
|------------------------------------------------------------------------------------------------------------|-----------------------------|---------------------------------|-----------------------------------------|----------------------------------|
|                                                                                                            | Hydrophilic/Non-hydrophilic | Weight average molecular weight | Tertiary amino group equivalent (eq/kg) | Polysiloxane segment content (%) |
| Production Example 4-1                                                                                     | Hydrophilic                 | 75,000                          | 0.66                                    | 3.2                              |
| Production Example 4-2                                                                                     | Hydrophilic                 | 71,000                          | 0.75                                    | 2.0                              |
| Production Example 4-3                                                                                     | Hydrophilic                 | 77,000                          | 1.22                                    | 1.2                              |
| Production Example 4b                                                                                      | Non-hydrophilic             | 72,000                          | Not contained                           | Not contained                    |
| Production Example 5b                                                                                      | Non-hydrophilic             | 84,000                          | 0.68                                    | Not contained                    |

40 Examples 3-1 to 3-3 and Comparative Examples 1b to 2b of Third Present Invention

45 Dispersion processing was applied for 24 hours by a ball mill with a high density alumina ball (3.5 g/ml) using each of the resin solutions obtained by the above-described Production Examples 3-1 to 3-3, 4b, and 5b and a zeolite (manufactured by Sun Zeolite Kogyo K.K.) with each combination (based on mass) shown in Table 8-1. And the contents after the dispersion were taken out through a 100 mesh sieve made of a polyester resin to obtain each resin composition in a liquid state comprising a resin solution and a zeolite.

TABLE 8-1

Preparation of resin compositions of Examples and Comparative Examples with regard to the third present invention [mass parts]

|                                          | Example 3-1 | Example 3-2 | Example 3-3 | Comparative Example 1b | Comparative Example 2b |
|------------------------------------------|-------------|-------------|-------------|------------------------|------------------------|
| Resin solution of Production Example 3-1 | 100         |             |             |                        |                        |
| Resin solution of Production Example 3-2 |             | 100         |             |                        |                        |
| Resin solution of Production Example 3-3 |             |             | 100         |                        |                        |
| Resin solution of Production Example 4b  |             |             |             | 100                    |                        |
| Resin solution of Production Example 5b  |             |             |             |                        | 100                    |

TABLE 8-1-continued

| Preparation of resin compositions of Examples and Comparative Examples with regard to the third present invention [mass parts] |             |             |             |                        |                        |
|--------------------------------------------------------------------------------------------------------------------------------|-------------|-------------|-------------|------------------------|------------------------|
|                                                                                                                                | Example 3-1 | Example 3-2 | Example 3-3 | Comparative Example 1b | Comparative Example 2b |
| Zeolite                                                                                                                        | 10          | 15          | 20          | 10                     | 20                     |
| Solvent (MEK/DMF = 7/3)                                                                                                        | 70          | 85          | 100         | 70                     | 100                    |

Examples 4-1 to 4-3 and Comparative Examples 1b to 2b of Fourth Present Invention

Dispersion processing was applied for 24 hours by a ball mill with a high density alumina ball (3.5 g/ml) using each of the resin solutions obtained by the above-described Production Examples 4-1 to 4-3, 4b, and 5b and a zeolite (manufactured by Sun Zeolite Kogyo K.K.) with each combination shown in Table 8-2. And the contents after the dispersion were taken out through a 100 mesh sieve made of a polyester resin to obtain each resin composition in a liquid state comprising a resin solution and a zeolite.

Good: No blocking property was observed.  
Fair: The blocking property was slightly observed.  
Poor: The blocking property was observed.

<Water Resistance>

Each resin film formed from each resin composition of Examples 4-1 to 4-3 and Comparative Examples 1b and 2b was cut in a shape having a thickness of 20  $\mu\text{m}$  and a longitudinal length of 5 cm  $\times$  a transversal length of 1 cm and immersed in water having a temperature of 25° C. for 12 hours, and the coefficient of expansion (%) in the longitudinal direction of the immersed film was measured and calculated by measuring the longitudinal length of the film after the

TABLE 8-2

| Preparation of resin compositions of Examples and Comparative Examples with regard to the fourth present invention [mass parts] |             |             |             |                        |                        |
|---------------------------------------------------------------------------------------------------------------------------------|-------------|-------------|-------------|------------------------|------------------------|
|                                                                                                                                 | Example 4-1 | Example 4-2 | Example 4-3 | Comparative Example 1b | Comparative Example 2b |
| Resin solution of Production Example 4-1                                                                                        | 100         |             |             |                        |                        |
| Resin solution of Production Example 4-2                                                                                        |             | 100         |             |                        |                        |
| Resin solution of Production Example 4-3                                                                                        |             |             | 100         |                        |                        |
| Resin solution of Production Example 4b                                                                                         |             |             |             | 100                    |                        |
| Resin solution of Production Example 5b                                                                                         |             |             |             |                        | 100                    |
| Zeolite                                                                                                                         | 10          | 15          | 20          | 10                     | 20                     |
| Solvent (MEK/DMF = 7/3)                                                                                                         | 70          | 85          | 100         | 70                     | 100                    |

[Evaluation of Third Present Invention and Fourth Present Invention]

The following tests were carried out using each resin composition of Examples and Comparative Examples of the fourth present invention to check the usefulness of each of the obtained resin compositions provided by the fourth present invention. Release paper was applied with each resin composition having the formulation shown in Table 8-2 and dried by heating at 110° C. for 3 minutes to volatilize the solvent, and each resin film having a thickness of about 20  $\mu\text{m}$  was formed. The following items were evaluated using each resin film thus obtained and formed from each resin composition of Examples 4-1 to 4-3 and Comparative Examples 1b and 2b of the fourth present invention.

<Blocking Resistance (Sticking Resistance)>

Film faces of each resin film of Examples 4-1 to 4-3 and Comparative Examples 1b and 2b formed from each resin composition were placed face to face, thereafter the films were left at 40° C. for 1 day while a load of 0.29 MPa was applied thereon. After that, the blocking property of the films with the faces placed face to face was visually observed and evaluated according to the following criteria. And the obtained results are shown in Table 9 together.

immersion test and using the following equation. And the water resistance was evaluated by rating a film having a coefficient of expansion of 200% or less as "Good" and a film having a coefficient of expansion of more than 200% as "Poor". The obtained results are shown in Table 9.

$$\text{Coefficient of expansion (\%)} = (\text{Longitudinal length after test} / \text{Original longitudinal length}) \times 100$$

TABLE 9

|                        | Evaluation results (blocking resistance and water resistance) |                                                 |
|------------------------|---------------------------------------------------------------|-------------------------------------------------|
|                        | Blocking resistance                                           | Water resistance (Coefficient of expansion (%)) |
| Example 4-1            | Good                                                          | Good (143)                                      |
| Example 4-2            | Good                                                          | Good (151)                                      |
| Example 4-3            | Good                                                          | Good (164)                                      |
| Comparative Example 1b | Poor to Fair                                                  | Good (106)                                      |
| Comparative Example 2b | Fair to Good                                                  | Good (105)                                      |

<Effect on Removal of Iodine Ion and Cesium Ion>

An iodine ion and cesium ion-removing function of each of the obtained resin compositions provided by the third present invention and the fourth present invention was checked in the following manner. Using each resin composition of Examples

and Comparative Examples of the third present invention and the fourth present invention, release paper was applied with each resin composition and dried by heating at 110°C. for 3 minutes to volatilize the solvent, and each resin film having a thickness of about 20  $\mu\text{m}$  was formed. The effect on the removal of an iodine ion and a cesium ion was evaluated by the following method using each resin film thus obtained and formed from each resin composition of Examples and Comparative Examples of the third present invention and the fourth present invention.

(Preparation of Iodine Solution and Cesium Solution for Evaluation Test>

An iodine solution for the evaluation test was prepared by dissolving potassium iodide in ion exchanged pure water so that the solution had an iodine ion concentration of 200 mg/L (200 ppm). Moreover, a cesium solution for the evaluation test was prepared by dissolving cesium chloride in ion exchanged pure water so that the solution had a cesium ion concentration of 200 mg/L (200 ppm). In addition, when iodine ion and cesium ion can be removed, radioactive iodine and radioactive cesium can be removed naturally.

(Evaluation Results with Regard to Resin Composition of Example 3-1 of Third Present Invention)

In a mixed solution of 50 ml of the iodine solution prepared for the evaluation test previously and 50 ml of the cesium solution prepared for the evaluation test previously, 20 g of the resin film prepared using the hydrophilic resin composition of Example 3-1 was immersed (25°C.), and the iodine ion concentration and the cesium ion concentration in the solution were measured by an ion chromatograph (IC2001 manufactured by Tosoh Corporation) every time a predetermined time was elapsed. The measurement results are shown in Table 10, and it was confirmed that, as shown in Table 10, both of the iodine ion concentration and the cesium ion concentration in the solution were decreased every time a predetermined time was elapsed. The removing rates of the iodine ion and the cesium ion in the solution every time a predetermined time is elapsed are listed together with the iodine ion concentration and the cesium ion concentration. Moreover, the results are shown in FIG. 4 and FIG. 5.

TABLE 10

Evaluation results in the case where the resin composition film of Example 3-1 of the third present invention was used

| Immersion time (Hr) | Iodine ion                      |                   | Cesium ion                      |                   |
|---------------------|---------------------------------|-------------------|---------------------------------|-------------------|
|                     | Concentration in solution (ppm) | Removing rate (%) | Concentration in solution (ppm) | Removing rate (%) |
| 0                   | 100.0                           | —                 | 100.0                           | —                 |
| 1                   | 80.3                            | 19.7              | 53.8                            | 46.2              |
| 5                   | 51.6                            | 48.4              | 18.1                            | 81.9              |
| 15                  | 46.8                            | 53.2              | 7.5                             | 92.5              |
| 24                  | 41.5                            | 58.5              | 4.1                             | 95.9              |

(Evaluation Results with Regard to Resin Composition of Example 3-2 of Third Present Invention)

The iodine ion concentration and the cesium ion concentration in the solution every time a predetermined time was elapsed were measured in the same manner as in the case where the resin film prepared using the hydrophilic resin composition of Example 3-1 was used except that 20 g of the resin film prepared by the hydrophilic resin composition of Example 3-2 was used. The obtained results are shown in Table 11, FIG. 4, and FIG. 5 in the same manner as in the case of Example 3-1 described previously.

TABLE 11

Evaluation results in the case where the resin composition film of Example 3-2 of the third present invention as used

| Immersion time (Hr) | Iodine ion                      |                   | Cesium ion                      |                   |
|---------------------|---------------------------------|-------------------|---------------------------------|-------------------|
|                     | Concentration in solution (ppm) | Removing rate (%) | Concentration in solution (ppm) | Removing rate (%) |
| 0                   | 100.0                           | —                 | 100.0                           | —                 |
| 1                   | 71.3                            | 28.7              | 45.2                            | 54.8              |
| 5                   | 48.5                            | 51.5              | 12.2                            | 87.8              |
| 15                  | 41.7                            | 58.3              | 3.3                             | 96.7              |
| 24                  | 38.8                            | 61.2              | 1.5                             | 98.5              |

(Evaluation Results with Regard to Resin Composition of Example 3-3 of Third Present Invention)

The iodine ion concentration and the cesium ion concentration in the solution every time a predetermined time was elapsed were measured in the same manner as in the case where the resin film prepared using the hydrophilic resin composition of Example 3-1 was used except that 20 g of the resin film prepared by the hydrophilic resin composition of Example 3-3 was used. The obtained results are shown in Table 12, FIG. 4, and FIG. 5 in the same manner as in the case of Example 3-1 described previously.

TABLE 12

Evaluation results in the case where the resin composition film of Example 3-3 of the third present invention was used

| Immersion time (Hr) | Iodine ion                      |                   | Cesium ion                      |                   |
|---------------------|---------------------------------|-------------------|---------------------------------|-------------------|
|                     | Concentration in solution (ppm) | Removing rate (%) | Concentration in solution (ppm) | Removing rate (%) |
| 0                   | 100.0                           | —                 | 100.0                           | —                 |
| 1                   | 68.1                            | 31.9              | 41.7                            | 58.3              |
| 5                   | 38.8                            | 61.2              | 8.5                             | 91.5              |
| 15                  | 31.7                            | 68.3              | 2.2                             | 97.8              |
| 24                  | 28.6                            | 71.4              | 0.8                             | 99.2              |

(Evaluation Results with Regard to Resin Composition of Example 4-1 of Fourth Present Invention)

In a mixed solution of 50 ml of the iodine solution prepared for the evaluation test previously and 50 ml of the cesium solution prepared for the evaluation test previously, 20 g of the resin film prepared using the hydrophilic resin composition of Example 4-1 was immersed (25°C.), and the iodine ion concentration and the cesium ion concentration in the solution were measured by an ion chromatograph (IC2001 manufactured by Tosoh Corporation) every time a predetermined time was elapsed. The results are shown in Table 13, and it was confirmed that, as shown in Table 13, both of the iodine ion concentration and the cesium ion concentration in the solution were decreased every time a predetermined time was elapsed. The removing rates of the iodine ion and the cesium ion in the solution every time a predetermined time is elapsed are listed in Table 13 together with the iodine ion concentration and the cesium ion concentration. Moreover, the results are shown in FIG. 6 and FIG. 7.

TABLE 13

| Evaluation results in the case where the resin composition film of Example 4-1 of the fourth present invention was used |                                 |                   |                                 |                   |                   |
|-------------------------------------------------------------------------------------------------------------------------|---------------------------------|-------------------|---------------------------------|-------------------|-------------------|
| Immersion time (Hr)                                                                                                     | Iodine ion                      |                   | Cesium ion                      |                   | Removing rate (%) |
|                                                                                                                         | Concentration in solution (ppm) | Removing rate (%) | Concentration in solution (ppm) | Removing rate (%) |                   |
| 0                                                                                                                       | 100.0                           | —                 | 100.0                           | —                 |                   |
| 1                                                                                                                       | 81.7                            | 18.3              | 54.5                            | 45.5              |                   |
| 5                                                                                                                       | 53.2                            | 46.8              | 18.6                            | 81.4              |                   |
| 15                                                                                                                      | 48.8                            | 51.2              | 8.3                             | 91.7              |                   |
| 24                                                                                                                      | 43.3                            | 56.7              | 3.8                             | 96.2              |                   |

(Evaluation Results with Regard to Resin Composition of Example 4-2 of Fourth Present Invention)

The iodine ion concentration and the cesium ion concentration in the solution every time a predetermined time was elapsed were measured in the same manner as in the case where the resin film prepared using the hydrophilic resin composition of Example 4-1 was used except that 20 g of the resin film prepared using the hydrophilic resin composition of Example 4-2 was used. The obtained results are shown in Table 14, FIG. 6, and FIG. 7 in the same manner as in the case of Example 4-1 described previously. As a result thereof, it was confirmed that both of the iodine ion concentration and the cesium ion concentration in the solution were decreased every time a predetermined time was elapsed also in the case where the hydrophilic resin composition of Example 4-2 was used.

TABLE 14

| Evaluation results in the case where the resin composition film of Example 4-2 of the fourth present invention was used |                                 |                   |                                 |                   |                   |
|-------------------------------------------------------------------------------------------------------------------------|---------------------------------|-------------------|---------------------------------|-------------------|-------------------|
| Immersion time (Hr)                                                                                                     | Iodine ion                      |                   | Cesium ion                      |                   | Removing rate (%) |
|                                                                                                                         | Concentration in solution (ppm) | Removing rate (%) | Concentration in solution (ppm) | Removing rate (%) |                   |
| 0                                                                                                                       | 100.0                           | —                 | 100.0                           | —                 |                   |
| 1                                                                                                                       | 77.6                            | 22.4              | 46.7                            | 53.3              |                   |
| 5                                                                                                                       | 50.2                            | 49.8              | 12.0                            | 88.0              |                   |
| 15                                                                                                                      | 43.3                            | 56.7              | 4.5                             | 95.5              |                   |
| 24                                                                                                                      | 40.5                            | 59.5              | 1.8                             | 98.2              |                   |

(Evaluation Results with Regard to Resin Composition of Example 4-3 of Fourth Present Invention)

The iodine ion concentration and the cesium ion concentration in the solution every time a predetermined time was elapsed were measured in the same manner as in the case where the resin film prepared using the hydrophilic resin composition of Example 4-1 was used except that 20 g of the resin film prepared by the hydrophilic resin composition of Example 4-3 was used. The obtained results are shown in Table 15, FIG. 6, and FIG. 7 in the same manner as in the case of Example 4-1 described previously. As a result thereof, it was confirmed that both of the iodine ion concentration and the cesium ion concentration in the solution were decreased every time a predetermined time was elapsed also in the case where the hydrophilic resin composition of Example 4-3 was used.

TABLE 15

| Evaluation results in the case where the resin composition film of Example 4-3 of the fourth present invention was used |                                 |                   |                                 |                   |                   |
|-------------------------------------------------------------------------------------------------------------------------|---------------------------------|-------------------|---------------------------------|-------------------|-------------------|
| Immersion time (Hr)                                                                                                     | Iodine ion                      |                   | Cesium ion                      |                   | Removing rate (%) |
|                                                                                                                         | Concentration in solution (ppm) | Removing rate (%) | Concentration in solution (ppm) | Removing rate (%) |                   |
| 0                                                                                                                       | 100.0                           | —                 | 100.0                           | —                 |                   |
| 1                                                                                                                       | 70.2                            | 29.3              | 43.1                            | 56.9              |                   |
| 5                                                                                                                       | 41.2                            | 58.8              | 10.5                            | 89.5              |                   |
| 15                                                                                                                      | 33.5                            | 66.5              | 3.5                             | 96.5              |                   |
| 24                                                                                                                      | 30.2                            | 69.8              | 1.2                             | 98.8              |                   |

(Evaluation Results with Regard to Resin Composition of Comparative Example 1b of Third Present Invention and Fourth Present Invention)

The iodine ion concentration and the cesium ion concentration in the solution were measured every time a predetermined time was elapsed in the same manner as in the case where the resin film prepared using the hydrophilic resin composition of Example 4-1 except that 20 g of the resin film prepared by the non-hydrophilic resin composition of Comparative Example 1b was used. The obtained results are shown in Table 16, FIG. 8, and FIG. 9 in the same manner as in the case of Example 4-1 described previously. As clearly understood from these results, the superiority of the removing performance of the iodine ion and the cesium ion in Examples of the third present invention and the fourth present invention was confirmed.

TABLE 16

| Evaluation results in the case where the resin composition film of Comparative Example 1b was used |                                 |                   |                                 |                   |                   |
|----------------------------------------------------------------------------------------------------|---------------------------------|-------------------|---------------------------------|-------------------|-------------------|
| Immersion time (Hr)                                                                                | Iodine ion                      |                   | Cesium ion                      |                   | Removing rate (%) |
|                                                                                                    | Concentration in solution (ppm) | Removing rate (%) | Concentration in solution (ppm) | Removing rate (%) |                   |
| 0                                                                                                  | 100.0                           | —                 | 100.0                           | —                 |                   |
| 1                                                                                                  | 98.8                            | 1.2               | 99.0                            | 1.0               |                   |
| 5                                                                                                  | 98.5                            | 1.5               | 98.8                            | 1.2               |                   |
| 15                                                                                                 | 98.1                            | 1.9               | 98.0                            | 2.0               |                   |
| 24                                                                                                 | 97.5                            | 2.5               | 97.4                            | 2.6               |                   |

(Evaluation Results with Regard to Resin Composition of Comparative Example 2b of Third Present Invention and Fourth Present Invention)

The iodine ion concentration and the cesium ion concentration in the solution were measured every time a predetermined time was elapsed in the same manner as in the case where the resin film prepared using the hydrophilic resin composition of Example 4-1 except that 20 g of a resin film prepared by the non-hydrophilic resin composition of Comparative Example 2b was used. The obtained results are shown in Table 17, FIG. 8, and FIG. 9 in the same manner as in the case of Example 4-1 described previously. As a result thereof, although the removing rates of the iodine ion and the cesium ion were improved more in the case where the non-hydrophilic resin composition of Comparative Example 2b was used than in the case where the non-hydrophilic resin composition of Comparative Example 1b was used, the superiority of the removing performance of the iodine ion and the cesium ion in Examples of the third present invention and the fourth present invention was confirmed.

TABLE 17

| Evaluation results in the case where the resin composition film of Comparative Example 2b was used |                                 |                   |                                 |                   |                   |
|----------------------------------------------------------------------------------------------------|---------------------------------|-------------------|---------------------------------|-------------------|-------------------|
| Immersion time (Hr)                                                                                | Iodine ion                      |                   | Cesium ion                      |                   | Removing rate (%) |
|                                                                                                    | Concentration in solution (ppm) | Removing rate (%) | Concentration in solution (ppm) | Removing rate (%) |                   |
| 0                                                                                                  | 100.0                           | —                 | 100.0                           | —                 |                   |
| 1                                                                                                  | 98.1                            | 1.9               | 97.8                            | 2.2               |                   |
| 5                                                                                                  | 97.5                            | 2.5               | 96.3                            | 3.7               |                   |
| 15                                                                                                 | 95.7                            | 4.3               | 95.5                            | 4.5               |                   |
| 24                                                                                                 | 96.1                            | 3.9               | 95.1                            | 4.9               |                   |

## Industrial Applicability

As an application example of the first present invention and the second present invention, radioactive cesium in liquid and/or a solid matter can be processed simply and at low cost, furthermore the removing processing of radioactive cesium can be applied without the need for an energy source such as electricity, therefore it becomes possible to remove a radioactive substance present in liquid or a solid matter which radioactive substance has been a problem recently simply and economically by carrying out the novel method for removing radioactive cesium, and thus the utilization can be expected.

Particularly, by the technique of the first present invention, the removed radioactive cesium is quickly taken in the first hydrophilic resin composition comprising: a first hydrophilic resin having a hydrophilic segment; and a zeolite and can stably be immobilized, furthermore since the main component of the first hydrophilic resin composition is a resin composition, the volume reduction of radioactive waste can be achieved as necessary, therefore the problem that radioactive waste produced after the removing processing of radioactive substances becomes huge can be reduced, the practical value is extremely high, and the utilization can be expected.

Moreover, by the second present invention, it becomes possible to realize, in addition to the effect obtained by the above-described first present invention, the water resistance and the blocking resistance (sticking resistance) of the surface brought about by the presence of a polysiloxane segment by introducing the polysiloxane segment in the structure of the second hydrophilic resin having a hydrophilic segment, and therefore the utilization can be expected from the point of realizing the water resistance and the blocking resistance.

As an application example of the third present invention and the fourth present invention, radioactive iodine and radioactive cesium in a radioactive waste liquid and/or a radioactive solid matter can be removed simply and at low cost, and furthermore without the need for an energy source such as electricity, therefore it becomes possible to remove radioactive substances present in a mixed state in liquid or a solid matter which radioactive substances have been a problem recently simply and economically by carrying out the novel method for simultaneously removing radioactive iodine and radioactive cesium, and thus the practical value is extremely high.

Particularly, by the technique of the third present invention, the removed radioactive iodine and radioactive cesium are taken in the third hydrophilic resin composition comprising: a third hydrophilic resin having a particular structure; and a zeolite and can stably be immobilized, furthermore since the main component of the third hydrophilic resin composition is a resin composition, the volume reduction of radioactive waste can be achieved as necessary, therefore the problem in large amounts of radioactive waste produced after the remov-

ing processing of radioactive substances can be reduced, and the utilization can be expected.

Moreover, by the fourth present invention, it becomes possible to realize, in addition to the effect obtained by the above-described third present invention, the water resistance and the blocking resistance (sticking resistance) of the resin surface brought about by the presence of a polysiloxane segment and to improve the practicability in the case where the removing processing is applied using the film or the like by using the fourth hydrophilic resin composition comprising a fourth hydrophilic resin introducing, in addition to a hydrophilic segment and a tertiary amino group forming an ion bond with radioactive iodine, a polysiloxane segment further in the structure thereof, therefore the problem in radioactive waste produced after the removing processing of radioactive substances can be reduced, and the utilization can be expected.

The invention claimed is:

1. A method for removing radioactive cesium applying removal processing to radioactive cesium in a radioactive waste liquid and/or a radioactive solid matter using a hydrophilic resin composition comprising a hydrophilic resin and a zeolite,

wherein the hydrophilic resin composition comprises at least one hydrophilic resin selected from the group consisting of a hydrophilic polyurethane resin, a hydrophilic polyurea resin, and a hydrophilic polyurethane-polyurea resin each having a hydrophilic segment; and the hydrophilic resin composition comprises the zeolite dispersed therein in a ratio of at least 1 to 200 mass parts relative to 100 mass parts of the hydrophilic resin.

2. A method for removing radioactive cesium applying removal processing to radioactive cesium present in a radioactive waste liquid and/or a radioactive solid matter using a hydrophilic resin composition comprising a hydrophilic resin and a zeolite,

wherein the hydrophilic resin comprises at least one selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a polysiloxane segment; and

the hydrophilic resin composition comprises the zeolite dispersed therein in a ratio of at least 1 to 200 mass parts relative to 100 mass parts of the hydrophilic resin.

3. The method for removing radioactive cesium according to claim 2, wherein the hydrophilic resin is a resin formed from, as a part of a raw material, a compound having at least one active hydrogen-containing group and a polysiloxane segment in the same molecule.

4. The method for removing radioactive cesium according to claim 1, wherein the hydrophilic segment is a polyethylene oxide segment.

5. The method for removing radioactive cesium according to claim 1, wherein the zeolite is a compound represented by the following general formula (1):



[where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number of from 1 to 18, and  $n$  is a number of from 1 to 70].

6. A hydrophilic resin composition for removing radioactive cesium having a function capable of immobilizing radioactive cesium in liquid and/or a solid matter,

wherein the hydrophilic resin composition comprises a hydrophilic resin and a zeolite;

## 51

the hydrophilic resin is a resin having a hydrophilic segment, the resin being insoluble to water and hot water; and

the zeolite is dispersed in the hydrophilic resin composition in a ratio of at least 1 to 200 mass parts relative to 100 mass parts of the hydrophilic resin.

7. A hydrophilic resin composition for removing radioactive cesium having a function capable of immobilizing radioactive cesium in liquid and/or a solid matter,

wherein the hydrophilic resin composition comprises a 10 hydrophilic resin and a zeolite;

the hydrophilic resin is at least one selected from the group consisting of a hydrophilic polyurethane resin, a hydrophilic polyurea resin, and a hydrophilic polyurethane-polyurea resin each having a hydrophilic segment and each obtained by reacting an organic polyisocyanate with a high molecular weight hydrophilic polyol and/or polyamine being a hydrophilic component; and the zeolite is dispersed in the hydrophilic resin composition in a ratio of at least 1 to 200 mass parts relative to 20 100 mass parts of the hydrophilic resin.

8. A hydrophilic resin composition for removing radioactive cesium exhibiting a function capable of immobilizing radioactive cesium in liquid and/or a solid matter,

wherein the hydrophilic resin composition comprises a 25 hydrophilic resin and a zeolite;

the hydrophilic resin is a resin having a hydrophilic segment and a polysiloxane segment and obtained by reacting, as a part of a raw material, a compound having at least one active hydrogen-containing group and a polysiloxane segment in the same molecule, the resin being insoluble to water and hot water; and

the zeolite is dispersed in the hydrophilic resin composition in a ratio of at least 1 to 200 mass parts relative to 30 100 mass parts of the hydrophilic resin.

9. A hydrophilic resin composition for removing radioactive cesium exhibiting a function capable of immobilizing radioactive cesium in liquid and/or a solid matter,

wherein the hydrophilic resin composition comprises a 35 hydrophilic resin and a zeolite;

the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a polysiloxane segment, and each obtained by reacting an organic polyisocyanate, a high molecular weight hydrophilic polyol and/or polyamine being a hydrophilic component, and a compound having at least one active hydrogen-containing group and a polysiloxane segment in the same molecule; and

the zeolite is dispersed in the hydrophilic resin composition in a ratio of at least 1 to 200 mass parts relative to 40 100 mass parts of the hydrophilic resin.

10. The hydrophilic resin composition for removing radioactive cesium according to claim 6, wherein the hydrophilic segment is a polyethylene oxide segment.

11. The hydrophilic resin composition for removing radioactive cesium according to claim 6, wherein the zeolite is a compound represented by the following general formula (1):



[where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number selected from 1 to 18, and  $n$  is a number selected from 1 to 70].

12. A method for removing radioactive iodine and radioactive cesium applying removal processing to both of radio-

## 52

active iodine and radioactive cesium in a radioactive waste liquid and/or a radioactive solid matter using a hydrophilic resin composition comprising a hydrophilic resin and a zeolite,

wherein the hydrophilic resin comprises at least one hydrophilic resin selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a tertiary amino group; and

the hydrophilic resin composition comprises the zeolite dispersed therein in a ratio of at least 1 to 200 mass parts relative to 100 mass parts of the hydrophilic resin.

13. The method for removing radioactive iodine and radioactive cesium according to claim 12, wherein the hydrophilic resin is a resin formed from, as a part of a raw material, a polyol having at least one tertiary amino group or a polyamine having at least one tertiary amino group.

14. A method for removing radioactive iodine and radioactive cesium applying removal processing to both of radioactive iodine and radioactive cesium present in a radioactive waste liquid and/or a radioactive solid matter using a hydrophilic resin composition comprising a hydrophilic resin and a zeolite,

wherein the hydrophilic resin comprises at least one selected from the group consisting of a hydrophilic polyurethane resin, a hydrophilic polyurea resin, and a hydrophilic polyurethane-polyurea resin each having a hydrophilic segment and further each having, in the main chain and/or a side chain in the structure thereof, a tertiary amino group and a polysiloxane segment; and the hydrophilic resin composition comprises the zeolite dispersed therein in a ratio of at least 1 to 200 mass parts relative to 100 mass parts of the hydrophilic resin.

15. The method for removing radioactive iodine and radioactive cesium according to claim 14, wherein the hydrophilic resin is a resin formed from, as a part of a raw material, a polyol having at least one tertiary amino group or a polyamine having at least one tertiary amino group, and a compound having at least one active hydrogen-containing group and a polysiloxane segment in the same molecule.

16. The method for removing radioactive iodine and radioactive cesium according to claim 12, wherein the hydrophilic segment is a polyethylene oxide segment.

17. The method for removing radioactive iodine and radioactive cesium according to claim 12, wherein the zeolite is a compound represented by the following general formula (1):



[where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number selected from 1 to 18, and  $n$  is a number selected from 1 to 70].

18. A hydrophilic resin composition for removing radioactive iodine and radioactive cesium having a function capable of immobilizing both of radioactive iodine and radioactive cesium in liquid and/or a solid matter,

wherein the hydrophilic resin composition comprises a hydrophilic resin and a zeolite; the hydrophilic resin is a resin having a hydrophilic segment, having, in the molecular chain, a tertiary amino group, and formed from, as a part of a raw material, a polyol having at least one tertiary amino group or a polyamine having at least one tertiary amino group, the resin being insoluble to water and hot water; and

the zeolite is dispersed in the hydrophilic resin composition in a ratio of at least 1 to 200 mass parts relative to 100 mass parts of the hydrophilic resin.

**19.** A hydrophilic resin composition for removing radioactive iodine and radioactive cesium exhibiting a function capable of immobilizing both of radioactive iodine and radioactive cesium in liquid and/or a solid matter,

wherein the hydrophilic resin composition comprises a hydrophilic resin and a zeolite;

the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a tertiary amino group, and each obtained by reacting an organic polyisocyanate, a high molecular weight hydrophilic polyol and/or polyamine being a hydrophilic component, and a compound having at least one active hydrogen-containing group and at least one tertiary amino group in the same molecule; and the zeolite is dispersed in the hydrophilic resin composition in a ratio of at least 1 to 200 mass parts relative to 100 mass parts of the hydrophilic resin.

**20.** A hydrophilic resin composition for removing radioactive iodine and radioactive cesium exhibiting a function capable of immobilizing both of radioactive iodine and radioactive cesium in liquid and/or a solid matter,

wherein the hydrophilic resin composition comprises a hydrophilic resin and a zeolite;

the hydrophilic resin is a resin having a hydrophilic segment, having, in the molecular chain, a tertiary amino group and a polysiloxane segment, and obtained by reacting a polyol having at least one tertiary amino group or a polyamine having at least one tertiary amino group with a compound having at least one active hydrogen-containing group and a polysiloxane segment in the same molecule, the resin being insoluble to water and hot water; and

the zeolite is dispersed in the hydrophilic resin composition in a ratio of at least 1 to 200 mass parts relative to 100 mass parts of the hydrophilic resin.

**21.** A hydrophilic resin composition for removing radioactive iodine and radioactive cesium exhibiting a function capable of immobilizing both of radioactive iodine and radioactive cesium in liquid and/or a solid matter,

wherein the hydrophilic resin composition comprises a hydrophilic resin and a zeolite;

the hydrophilic resin is at least one selected from the group consisting of a hydrophilic polyurethane resin, a hydrophilic polyurea resin, and a hydrophilic polyurethane-polyurea resin each having a hydrophilic segment, further each having, in the main chain and/or a side chain in the structure thereof, a tertiary amino group and a polysiloxane segment, and each obtained by reacting an organic polyisocyanate, a high molecular weight hydrophilic polyol and/or polyamine being a hydrophilic component, a compound having at least one active hydrogen-containing group and at least one tertiary amino group in the same molecule, and a compound having at least one active hydrogen-containing group and a polysiloxane segment in the same molecule; and

the zeolite is dispersed in the hydrophilic resin composition in a ratio of at least 1 to 200 mass parts relative to 100 mass parts of the hydrophilic resin.

**22.** The hydrophilic resin composition for removing radioactive iodine and radioactive cesium according to claim **18**, wherein the hydrophilic segment of the hydrophilic resin is a polyethylene oxide segment.

**23.** The hydrophilic resin composition for removing radioactive iodine and radioactive cesium according to claim **18**, wherein the zeolite is a compound represented by the following general formula (1):



[where, in the formula (1),  $M^{2+}$  is any one of  $Ca^{2+}$ ,  $Mn^{2+}$ ,  $Ba^{2+}$ , and  $Mg^{2+}$ ,  $M^+$  is any one of  $Na^+$ ,  $K^+$ , and  $Li^+$ ,  $m$  is a number of from 1 to 18, and  $n$  is a number of from 1 to 70].

\* \* \* \* \*